

[54] FERROMAGNETIC TONER CONTAINING  
WATER-SOLUBLE OR  
WATER-SOLUBILIZABLE RESIN(S)

[75] Inventor: Emery John Gorondy, Wilmington, Del.

[73] Assignee: E. I. Du Pont de Nemours and Company, Wilmington, Del.

[21] Appl. No.: 672,554

[22] Filed: Mar. 31, 1976

[51] Int. Cl.<sup>2</sup> ..... H01F 1/00; H01F 1/26;  
G03G 9/08

[52] U.S. Cl. ..... 252/62.1 P; 8/2;  
96/1 SD; 106/15 R; 106/15 FP; 106/16;  
252/8.1; 252/8.6; 252/62.54; 252/301.21;  
346/74.1; 424/31; 424/32; 424/33; 427/18;  
427/27; 427/47; 427/127

[58] Field of Search ..... 252/62.1 P, 62.1 L,  
252/62.1 R, 62.54, 316, 8.1, 8.6, 301.21;  
346/74.1; 8/2; 427/18, 27, 47, 127; 96/1 SD;  
424/31, 32, 33; 106/15 R, 15 FP, 16

[56] References Cited

U.S. PATENT DOCUMENTS

2,890,968 6/1959 Giaimo ..... 252/62.54 X  
2,971,916 2/1961 Schlekher et al. ..... 428/407 X

|           |         |                     |              |
|-----------|---------|---------------------|--------------|
| 3,052,564 | 9/1962  | Kulesza .....       | 427/47       |
| 3,155,531 | 11/1964 | Fauser et al. ....  | 252/62.1 L X |
| 3,239,465 | 3/1966  | Rheinfrank .....    | 96/1.5 X     |
| 3,345,294 | 10/1967 | Cooper .....        | 252/62.1 P   |
| 3,377,286 | 4/1968  | Stricklin .....     | 252/62.1 P   |
| 3,454,347 | 7/1969  | Leimbacher .....    | 8/34 X       |
| 3,558,492 | 1/1971  | Proskow .....       | 252/62.1 P X |
| 3,573,979 | 12/1971 | Honjo .....         | 252/62.54 X  |
| 3,627,682 | 12/1971 | Hall et al. ....    | 252/62.54    |
| 3,781,903 | 12/1973 | Jeffers et al. .... | 118/637 X    |
| 3,782,895 | 1/1974  | Goorhuis .....      | 8/2          |

FOREIGN PATENT DOCUMENTS

144,460 3/1962 U.S.S.R. .... 8/2

Primary Examiner—Harris A. Pitlick

[57] ABSTRACT

Ferromagnetic toner which is useful in magnetic printing processes and devices for printing a variety of substrates, including textiles, such as fabric and yarn, film, paper, metal and wood, which toner comprises a ferromagnetic component, a dye and/or chemical treating agent and a readily fusible water-soluble or -solubilizable, preferably thermoplastic, resin which substantially encapsulates the ferromagnetic component and the dye and/or treating agent.

54 Claims, No Drawings

**FERROMAGNETIC TONER CONTAINING  
WATER-SOLUBLE OR WATER-SOLUBILIZABLE  
RESINS(S)**

**BACKGROUND OF THE INVENTION**

**1. Field of the Invention**

This invention relates to ferromagnetic toners which are useful in magnetic printing processes and devices.

**2. Description of the Prior Art**

One form of copying process in wide usage is the electrostatic copying process. Operation of such a process may provide difficulties in that large black areas may not be amenable to copying and the document to be copied may have to be reimaged each time a copy is made. The overcoming of these difficulties may be economically prohibitive. It is well known that audio signals and digital data can be recorded on magnetic materials. Magnetic field configurations in the form of alphabetical characters and pictures can also be produced by selective magnetization or demagnetization of the surface of a ferromagnetic chromium dioxide film. The resultant fields are strong enough to attract and hold small magnetic particles such as iron powder. The development, that is, the making visible, of such a latent magnetic image can be effected by contacting the image surface with a magnetic developer, usually referred to as a magnetic toner, consisting of ferromagnetic particles and pigments encapsulated in a thermoplastic resin binder. Such a development process is commonly known as decoration of the latent magnetic image. The developed image can then be transferred to and fixed on paper, thus providing a black-on-white copy of the latent image. Operation of such magnetic processes, however, may not be completely free of difficulties. For example, since most magnetic toner particles are attracted by both electrostatic and magnetic fields, any electrostatic field which is present on the magnetic surface may interfere with the interaction of the magnetic image and the magnetic toner particles. More specifically, a portion of the magnetic surface other than that containing the magnetic image may attract enough magnetic toner particles to render unsatisfactory the paper print which subsequently is produced.

There is extensive prior art in the fields of magnetic recording tapes and thermomagnetic recording. U.S. Pat. No. 3,476,595 discloses a magnetic recording tape which is coated with a thin layer of a cured complex of silica and a preformed organic polymer containing a plurality of alcoholic hydroxy groups. The disclosure includes coated, ferromagnetic, chromium dioxide, magnetic recording tapes. Discussions of acicular chromium dioxide and magnetic recording members bearing a layer of such material may also be found in U.S. Pat. Nos. 2,956,955 and 3,512,930. U.S. Pat. No. 3,554,798 discloses a magnetic recording member which is relatively transparent to light (transmits 5 to 95%) and which includes a plurality of discrete areas of hard magnetic particulate material supported thereon and bound thereto. A magnetically hard material is a material which is permanently magnetizable below the Curie point of the material, as opposed to a magnetically soft material which is substantially non-permanently magnetizable under similar conditions below the Curie point of the material. Chromium dioxide is disclosed as an example of a hard magnetic material. Decoration of the image may be effected by means of a magnetic pigment, for example, a dilute, alkyd-oil/water emulsion, carbon

black-based printing ink. U.S. Pat. No. 3,522,090 is similar in disclosure to U.S. Pat. No. 3,554,798 in that it also discloses a light-transparent recording member. However, it also discloses that the magnetic material which is capable of magnetization to a hard magnetic state (on the recording member) may have a coating of a reflective material which is so disposed that the magnetic material is shielded from exposing radiation while the adjacent uncoated portion of the recording member transmits 10 to 90% of the exposing radiation. The reflective coating can be a metallic reflector, such as aluminum, or a diffuse reflective pigment, such as titanium oxide. U.S. Pat. No. 3,555,556 discloses a direct thermomagnetic recording process wherein the document to be copied is imaged by light which passes through the document. U.S. Pat. No. 3,555,557 discloses a reflex thermomagnetic recording process wherein the light passes through the recording member and reflects off of the document which is to be copied. Thus, in the direct process, the document must be transparent but the recording member need not be transparent, whereas in the reflex process, the recording member must be transparent but the document need not be transparent. For the recording member to be transparent, it must have regions which are free of magnetic particles, that is, a non-continuous magnetic surface must be used.

U.S. Pat. No. 3,627,682 discloses ferromagnetic toner particles, for developing magnetic images, that include binary mixtures of a magnetically hard material and a magnetically soft material, an encapsulating resin and, optionally, carbon black or black or colored dyes to provide a blacker or colored copy. "Nigrosine" SSB is disclosed as an example of a black dye. The encapsulating resin aids transfer of the decorated magnetic image to paper and can be heated, pressed or vapor softened to adhere or fix the magnetic particles to the surface fibers of the paper. Ferromagnetic toner particles of the type disclosed in U.S. Pat. No. 3,627,682 are disclosed as being useful in the dry thermomagnetic copying process of U.S. Pat. No. 3,698,005. The latter patent discloses such a dry thermomagnetic copying process wherein the magnetic recording member is coated with a polysilicic acid. The use of the polysilicic acid coating on the recording member is particularly useful when the magnetic material on the recording member comprises a plurality of discrete areas of particulate magnetic material because a greater number of clean copies can be produced. The polysilicic acid, which is relatively non-conductive, exhibits good non-stick properties. Thus, toner particles which are held to the surface of the recording member by nonmagnetic forces can be easily removed without removing the toner particles which are held to the surface of the recording member by magnetic forces. U.S. Pat. No. 2,826,634 discloses the use of iron or iron oxide magnetic particles, either alone or encapsulated in low-melting resins, for developing magnetic images. Such toners have been employed to develop magnetic images recorded on magnetic tapes, films, drums and printing plates.

Japanese Pat. No. 70/52044 discloses a method which comprises adhering iron particles bearing a photosensitive diazonium compound onto an electrophotographic material to form an image, transferring the image onto a support having a coupler which is able to form an azo dye by reaction with the diazonium compound, reacting the diazonium compound and the coupler and thereafter removing the iron particles. U.S. Pat. No. 3,530,794 discloses a magnetic printing arrangement wherein a

thin, flexible master sheet having magnetizable, character-representing, mirror-reversed printing portions is employed in combination with a rotary printing cylinder. The master sheet, which consists of a thin, flexible non-magnetizable layer, such as paper, is placed on top of and in contact with a layer of iron oxide or ferrite which is adhesively attached to a base sheet. The combined layer and base sheet are imprinted, for example, by the impact of type faces, so that mirror-reversed, character representing portions of the iron oxide layer adhere to the non-magnetizable layer, thus forming magnetizable printing portions on same. Thereafter, the printing portions are magnetized and a magnetizable toner powder, such as iron powder, is applied to and adheres to the magnetized printing portions. The powder is then transferred from the printing portions to a copy sheet and permanently attached thereto, for example, by heating. U.S. Pat. No. 3,052,564 discloses a magnetic printing process employing a magnetic ink consisting of granules of iron coated with a colored or uncolored thermoplastic wax composition. The magnetic ink is employed in effecting the transfer of a printed record, using magnetic means, to paper. U.S. Pat. No. 3,735,416 discloses a magnetic printing process wherein characters or other data to be printed are formed on a magnetic recording surface by means of a recording head. A magnetic toner which is composed of resin-coated magnetic particles is employed to effect transfer of the characters or other data from the recording surface to a receiving sheet. U.S. Pat. No. 3,250,636 discloses a direct imaging process and apparatus wherein a uniform magnetic field is applied to a ferromagnetic imaging layer; the magnetized, ferromagnetic imaging layer is exposed to a pattern of heat conforming to the shape of the image to be reproduced, the heat being sufficient to raise the heated portions of the layer above the Curie point temperature of the ferromagnetic imaging layer so as to form a latent magnetic image on the imaging layer; the latent magnetic image is developed by depositing a finely divided magnetically attractable material on the surface of the ferromagnetic imaging layer; the imaging layer is uniformly heated above its Curie point temperature after the development to uniformly demagnetize it; and, finally, the loosely adhering magnetically attractable material is transferred from the imaging layer to a transfer layer.

German Pat. No. 2,452,530 discloses electrophotographic toners comprising a magnetic component coated with an organic substance containing a dye which vaporizes at 100° to 220° C, preferably 160° to 200° C, at atmospheric pressure. The magnetic component is preferably granular iron and/or iron oxide and the coating is a water-insoluble polymer melting at about 150° C, e.g., polyamides, epoxy resins and cellulose ethers and esters. Both basic and disperse dyes can be used in the toners. The toners are from 1 to 10 microns in diameter and may also contain silicic acid as anti-static agent. Colored or black copies are formed by toner development of the latent image on a photo-conducting sheet of ZnO paper, followed by transfer of the dye in the vapor phase to a receiving sheet by application of heat and pressure.

#### OBJECTS AND SUMMARY OF THE INVENTION

Generally, only reddish-brown or black images can be obtained on paper using prior art ferromagnetic toners because of the dark hard magnetic components, for

example, the iron oxides ( $\gamma$ -Fe<sub>2</sub>O<sub>3</sub> or Fe<sub>3</sub>O<sub>4</sub>), and the dark soft magnetic components, for example, iron, employed therein; because the magnetic components are retained in and may be essential to the formation of the visible images; and because the magnetic components are bound to the paper by the encapsulating resins employed therein. It is an object of the present invention to provide a ferromagnetic toner which can be employed in magnetic printing processes and devices to print, in a broad range of colors, if desired, a variety of substrates, including textiles, such as fabric and yarn, film, paper, metal and wood. It is a further object to provide such a print which is substantially free of hard and soft magnetic components and encapsulating resin. Still another object is to provide a ferromagnetic toner from which the hard magnetic component and, if present, the soft magnetic component, and the encapsulating resin can be readily removed by means of an aqueous scour after the toner has been employed in a magnetic printing process and device. The term "textile" is intended to include any natural or synthetic material, such as natural and regenerated cellulose, cellulose derivatives, natural polyamides, such as wool, synthetic polyamides, polyesters, acrylonitrile polymers and mixtures thereof, which is suitable for spinning into a filament, fiber or yarn. The term "fabric" is intended to include any woven, knitted or nonwoven cloth comprised of natural or synthetic fibers, filaments or yarns.

In summary, the invention herein resides in a ferromagnetic toner comprising a ferromagnetic component, a dye and/or a chemical treating agent and a readily fusible, water-soluble or -solubilizable, preferably thermoplastic, resin which substantially encapsulates the ferromagnetic component and the dye and/or treating agent.

#### DETAILED DESCRIPTION OF THE INVENTION

The invention resides in a ferromagnetic toner comprising:

- (a) at least one ferromagnetic component;
- (b) at least one member of the group consisting of dye and chemical treating agent; and
- (c) a readily fusible, water-soluble or water-solubilizable resin which substantially encapsulates (a) and (b).

A preferred embodiment includes such toners comprising, based on the total weight of (a), (b) and (c), 14 to 83% of (a), 0.10 to 25% of (b) and 9 to 74% of (c) and having a resin to ferromagnetic component ratio of 0.11 to 3.3. An especially preferred embodiment is one wherein there is 55 to 70% of (a), 0.10 to 15% of (b) and 30 to 40% of (c) and which has a resin to ferromagnetic component ratio of 0.40 to 1.0.

The ferromagnetic component can consist of hard magnetic particles, soft magnetic particles or a binary mixture of hard and soft magnetic particles. The magnetically soft particles can be iron or another high-permeability, low-remanence material, such as iron carbonyl, certain of the ferrites, for example, (Zn, Mn)Fe<sub>2</sub>O<sub>4</sub>, or permalloys. The magnetically hard particles can be an iron oxide, preferably Fe<sub>3</sub>O<sub>4</sub>,  $\gamma$ -Fe<sub>2</sub>O<sub>3</sub>, other ferrites, for example, BaFe<sub>12</sub>O<sub>19</sub>, chi-iron carbide, chromium dioxide or alloys of Fe<sub>3</sub>O<sub>4</sub> and nickel or cobalt. As already indicated above, magnetically hard and magnetically soft particles are substances which are, respectively, permanently magnetizable and substantially non-permanently magnetizable under similar con-

ditions below the Curie point of the substances. A magnetically hard substance has a high-intrinsic coercivity, ranging from a few tens of oersteds (Oe), for example, 40 Oe, to as much as several thousand oersteds and a relatively high remanence (20 percent or more of the saturation magnetization) when removed from a magnetic field. Such substances are of low permeability and require high fields for magnetic saturation. Magnetically hard substances are used as permanent magnets for applications such as loud speakers and other acoustic transducers, in motors, generators, meters and instruments and as the recording layer in most magnetic tapes. A magnetically soft substance has low coercivity, for example, one oersted or less, high permeability, permitting saturation to be obtained with a small applied field, and exhibits a remanence of less than 5 percent of the saturation magnetization. Magnetically soft substances are usually found in solenoid cores, recording heads, large industrial magnets, motors and other electrically excited devices wherein a high flux density is required. Preferred soft magnetic substances include iron-based pigments, such as carbonyl iron, iron flakes and iron alloys.

Dyes which are useful in the ferromagnetic toners of this invention can be selected from virtually all of the compounds mentioned in the Colour Index, Vols. 1, 2 and 3, 3rd Edition, 1971. Such dyes are of a variety of chemical types; the choice of dye is determined by the nature of the substrate being printed. For example, pre-metallized dyes (1:1 and 2:1 dye:metal complexes) are suitable for synthetic polyamide fibers. The majority of such dyes are monoazo or disazo dyes; a lesser number are anthraquinone dyes. Such dyes can have or be free from water-solubilizing groups, such as sulfonic acid and carboxy groups, and sulfonamido groups. Acid wool dyes, including the monoazo, disazo and anthraquinone members of this class which bear water-solubilizing sulfonic acid groups, may also be suitable for synthetic polyamide textiles. Disperse dyes can be used for printing synthetic polyamide, polyester and regenerated cellulosic fibers. A common feature of such dyes is the absence of water-solubilizing groups. However, they are, for the most part, thermosoluble in synthetic polymers, notably polyesters, polyamides and cellulose esters. Disperse dyes include dyes of the monoazo, polyazo, anthraquinone, styryl, nitro, phthaloperinone, quinophthalone, thiazine and oxazine series and vat dyes in the leuco or oxidized form. For polyacrylonitrile and acid-modified polyester fibers, preference usually is given to cationic dyes containing a carbonium ion or a quaternary ammonium group. Cationic-disperse dyes, that is, water-insoluble salts of dye cations and selected arylsulfonate anions, are well-known in the art for dyeing acid-modified polyester and acrylic fibers. Cotton fibers can be printed with vat dyes and with fiber reactive dyes, including those which are employed for polyamide fibers. Other suitable dyes for cotton are the water-soluble and water-insoluble sulfur dyes. Water-swellable cellulosic fibers, or mixtures or blends thereof with synthetic fibers, can also be uniformly printed with water-insoluble disperse dyes using aqueous ethylene glycol or polyethylene glycol type solvents, as described in the art.

The amount of dye present in the ferromagnetic toners of this invention can vary over a wide range, for example, 0.1 to 25% by weight of the total weight of essential components (a), (b) and (c) in the toner. Partic-

ularly good results can be obtained when the amount is 0.1 to 15% by weight.

A wide variety of chemical treating agents, such as flame-retarding agents, biocides, ultraviolet light absorbers, fluorescent brighteners, dyeability modifiers and soil-release and water-proofing agents, are useful in the ferromagnetic toners of this invention. Such agents have utility on cotton, regenerated cellulose, wood pulp, paper, synthetic fibers, such as polyesters and 10 polyamides, and blends of cotton with polyester or polyamide. By dyeability modifier is meant a chemical substance that can be chemically or physically bound to the substrate, such as a fiber, to change the dyeability of the substrate, for example, the degree of dye fixation or 15 the type or class of dye that can be employed. A specific example of a useful dyeability modifier is a treating agent which provides printed chemical resists, that is, printed areas which remain unstained during a subsequent dyeing operation. Since many chemical treating 20 agents, including those of the aforesaid types, are well-known in the prior art, no further discussion thereof is necessary. The chemical treating agent in the toner can be present in the same amount as the dye, that is, 0.1 to 25%, preferably 0.1 to 15%, of the total weight of essential components (a), (b) and (c).

The resins which are useful in the ferromagnetic toners include any of the known, readily fusible, natural, modified natural or synthetic resins or polymers which are soluble or solubilizable in water, that is, either directly soluble in water or made soluble through a simple chemical treatment. The solubility in water must be such that the ferromagnetic component and the encapsulating resin can be removed from the substrate, after permanent fixation of the dye and/or chemical 30 treating agent, by an aqueous scour, in a short time, as will be described in greater detail hereinafter. Examples of solubilizable resins are those resins or polymers which contain salt-forming groups, which thereby render them soluble in an alkaline aqueous solution, and 35 those which can be hydrolyzed by acids or alkalis so as to become water-soluble. Exemplary of useful natural resins are rosin (also known as colophony) and modified derivatives thereof, such as rosin esterified with glycerin or pentaerythritol, dimerized and polymerized rosin, unsaturated or hydrated rosin and derivatives thereof and rosin, and derivatives thereof, which has been modified with phenolic or maleic resins. Other natural resins with properties similar to rosin, such as 40 dammar, copal, sandarak, shellac and talloel, can be successfully used in the ferromagnetic toners.

Examples of synthetic resins which are useful herein include vinyl polymers, such as polyvinyl alcohol and polyvinyl acetate copolymers; polyacrylic acid and polyacrylamide; methyl-, ethyl- and butyl methacrylate-methacrylic acid copolymers; styrene-maleic acid 45 copolymers; methyl vinyl ether-maleic acid copolymers; carboxyester lactone polymers; polyethylene oxide polymers; nonhardening phenolformaldehyde copolymers; polyester resins, such as linear polyesters prepared from dicarboxylic acids and alkylene glycols, for example, from phthalic, terephthalic, isophthalic or 50 sebacic acid and ethylene glycol; cellulose ethers, such as hydroxypropylcellulose; polyurethanes; and polyamides, such as those prepared from sebacic acid and hexamethylenediamine.

Resins used in the toners herein are preferably of the thermoplastic type in order to permit adhesion thereof to the substrate by melting or fusion. Particularly pre-

ferred resins herein are adducts of rosin, a dicarboxylic acid or anhydride, a polymeric fatty acid and an alkylene polyamide; hydroxypropylcellulose prepared by reacting 3.5 to 4.2 moles of propylene oxide per D-glucopyranosyl unit of the cellulose; and polyvinyl acetate copolymers having a free carboxy group content equivalent to 0.002 to 0.01 equivalent of ammonium hydroxide per gram of dry copolymer. The preferred resins possess a high electrical resistance for good transfer in an electrostatic field, have good infrared and steam fusion properties and do not interfere with penetration of the dye or chemical treating agent into the substrate during the final (permanent) fixation operation. Moreover, after the dye and/or chemical treating agent has been fixed within the substrate, the resin must be easily removable in an aqueous washing operation in a short time, for example, in less than five minutes at less than 100° C, preferably in less than 60 seconds at less than 90° C.

The ferromagnetic toners of this invention can be prepared by intimately mixing together, for example, by ball milling or by high frequency viscous milling, an aqueous solution or slurry containing the desired proportions of dye(s) and/or chemical treating agent(s), ferromagnetic component(s) and encapsulating resin and then spray-drying to remove the water. Particularly good results usually can be obtained by ball milling for 1-17 hours at about 60 percent by weight nonvolatiles content. The solution or dispersion resulting from ball milling is separated from the ceramic balls, sand or other grinding means, diluted with water and spray-dried at a nonvolatiles content of 10 to 40 percent by weight. Spray-drying is accomplished by conventional means, for example, by dropping the solution or dispersion onto a disk rotating at high speed or by using a conventional spray-drying nozzle, as described in the art. Spray-drying consists of atomizing the aqueous toner solution or dispersion into small droplets, mixing these with a gas, and holding the droplets in suspension in the gas until the water in the droplets evaporates and heat and surface tension forces cause the resin particles in each droplet to coalesce and encase the dye and/or treating agent included in the droplet. Most frequently, spray-drying is carried out with air as the gas for the drying step. The gas is heated sufficiently to remove the water and so that the many small particles in any one droplet formed during atomization can come together to form a small, hard, spherical toner particle which entraps any dye and/or treating agent initially included within that droplet.

By maintaining uniformity of dispersion of dye and resin in the water and by controlling solids concentration in the final dye-water mixture, the particle size of the toner can be controlled by the size of the droplet produced by the atomizing head in the spray-drying equipment. Moreover, by controlling the toner slurry feed rate, the viscosity of the toner slurry, the spray-drying temperature and the disc rpm for a disc atomizer, the pressure for a single-fluid nozzle atomizer or the pressure and air to feed ratio for a two-fluid nozzle atomizer, spherical toner particles having diameters within the range of 2 to 100 microns, preferably 10 to 25 microns, can be readily obtained. Toners passing a 200 mesh screen (U.S. Sieve Series), thus being less than 74 microns in the longest particle dimension, are especially useful.

Other suitable well known encapsulation processes can be employed to produce the ferromagnetic toners of

this invention. These include coacervation and interfacial polymerization techniques.

The relative amounts of resinous material and ferromagnetic material in the toner usually are determined by the desired adhesive and magnetic properties of the toner particle. Generally, the ratio of resinous material to ferromagnetic material is 0.11 to 3.3, preferably 0.40 to 1.0. The preferred ratio especially provides toners having good decoration, transfer and fusion properties.

It is to be understood that the ferromagnetic component, dye and/or chemical treating agent and encapsulating resin are essential components of the toners of this invention and the aforesaid percentages are based on the combined weights of these essential components. In some cases, it may be advisable to add one or more known chemical assistants to enhance the functional behavior of the ferromagnetic toner, for example, dispersing agents, surfactants and materials to promote dye and/or treating agent fixation in the substrate. Further examples of such chemical assistants include urea; latent oxidizing agents, such as sodium chlorate and sodium m-nitrobenzene sulfonate; latent reducing agents; acid or alkali donors, such as ammonium salts and sodium trichloroacetate; and dye carriers, usually present in amounts of 0.1 to 8% by weight based on the total toner weight, such as benzyl alcohol, benzanilide,  $\beta$ -naphthol, o-phenylphenol and butyl benzoate. Conventional commercial dispersing agents, such as the lignin sulfonates and salts of sulfonated naphthalene-formaldehyde condensates, can be employed. Such agents include "Polysol," a sodium salt of sulfonated lignin; "Reax," the sodium salts of sulfonated lignin derivatives; "Marasperse," a partially desulfonated sodium lignosulfonate; "Lignosol," sulfonated lignin derivatives; "Blancol," "Blancol" N and "Tamol," the sodium salt of sulfonated naphthalene-formaldehyde condensates; and "Daxad" 11 KLS and "Daxad" 15, the polymerized potassium and sodium salts, respectively, of alkyl naphthalenesulfonic acid. Other known useful auxiliary chemicals can assist in the prevention of "bleeding" of the dye pattern by preventing the swelling or coagulation of the resin. Exemplary of such auxiliary chemicals are starch, starch derivatives, sodium alginate and locust bean flour and its derivatives. Cationic surfactants, such as quaternary ammonium compounds, reduce the static propensity of the toner particles for the image-bearing magnetic film. Lower toner pickup in background or non-image areas can be achieved by incorporating such surfactants into the toner. Dimethyldistearylammonium chloride has been found to be particularly useful for this purpose. Still other auxiliary chemicals which may be present in the toner include known additives for improving the brightness and tintorial strength of the dyeing, for example, citric acid, which is commonly used with cationic dyes, and ammonium oxalate, which is commonly used with acid dyes.

A free-flow agent, usually present in an amount within the range 0.01 to 5% by weight, preferably 0.01 to 0.4% by weight, based on total toner weight, can be added to keep the individual toner particles from sticking together and to increase the bulk of the toner powder. This facilitates an even deposition of toner particles on the latent magnetic image. Free-flow or dispersing agents, such as microfine silica, alumina and fumed silica sold under the trade names "Quso" and "Cab-O-Sil," are useful.

The toners of this invention are especially useful in a process for magnetic printing comprising the steps of

forming a latent magnetic image on the surface of a magnetic printing member, developing the latent magnetic image by decoration with the ferromagnetic toner particles, transferring the toner-decorated image to a substrate, temporarily fixing the toner particles to the substrate, permanently fixing the dye and/or chemical treating agent to the substrate, and finally, removing the ancillary substances and any excess dye and/or agent from the substrate. The latent magnetic image can be developed by any convenient known method. Typical methods include cascade, magnetic brush, magnetic roll, powder cloud and dusting by hand. Cascade, magnetic brush, powder cloud and magnetic roll development are well known in the art.

Transfer of the ferromagnetic toner to the substrate can be accomplished either by magnetic, pressure or, preferably, by electrostatic means, that is, by applying a positive or negative potential to the backside of the substrate placed in contact with the toner-decorated latent magnetic image. The use of high pressure, for example, near 400 pounds per linear inch (about 70 kg per cm), generally results in shorter printing surface life, poorer transfer efficiency and poorer image definition on the substrate. Such problems are avoided by using electrostatic transfer means wherein there is no substantial amount of pressure between the printing surface and the substrate and, therefore, abrasion is minimized.

As mentioned hereinabove, the toners can be printed on all types of printable substrates. Particularly preferred are fabric substrates, especially those prepared from natural and regenerated cellulose, cellulose derivatives, wool and synthetic fibers, such as polyamides, polyesters and polyacrylics, and mixtures of any of these fabrics. Film substrates, for example, "Mylar" polyester film, are also preferred.

The ferromagnetic dye and/or chemical toner can be temporarily fixed to the substrate by melting it by the application of heat or by partially dissolving it in water, either in the form of an aqueous spray or as steam. Steam fusion at 100° C for 1 to 15 seconds at 1 atm pressure is particularly preferred.

Permanent fixation can be accomplished in any way which is consistent with the type of substrate and dye and/or chemical treating agent which are used. For example, dry-heat treatment, such as a Thermosol treatment, at 190° to 230° C for up to 100 seconds can be used to fix disperse dyes on polyester and mixed disperse-fiber reactive dyes on polyester-cotton. Moreover, high pressure steaming at pressures of 10 to 25 psig (0.7 to 1.76 kg per sq cm gauge) accelerates the fixation of disperse dyes on polyester and cellulose triacetate. Rapid disperse dye fixation can also be obtained by high-temperature steaming at 150 to 205° C for 4 to 8 minutes. High-temperature steaming provides the advantage of short treatment times without the need to use pressure seals.

Cottage-steaming and pressure-steaming can be used to fix cationic dyes to acid-modified acrylic and polyester fibers and to fix acid dyes, including premetalized dyes, to polyamide and wool fibers. Cottage-steaming uses saturated steam at a pressure of 1 to 7 psig (0.07 to 0.49 kg per sq cm gauge) and a relative humidity of 100%. There is no tendency to remove moisture from the fabric using saturated steam. As the fabric is initially contacted by the steam, a deposit of condensed water quickly forms on its cold surface. Such water serves various functions, such as swelling the fiber and activating the chemicals and dyes, thereby creating the condi-

tions necessary for their diffusion into the fiber. Rapid aging at 100° to 105° C for 15 to 45 minutes at 760 mm of pressure can be used to fix disperse dyes on cellulose acetate and cationic dyes on acrylic fibers.

Depending on the nature of the dye and/or chemical treating agent, it may also be necessary or desirable to treat the fabric with an aqueous solution before final fixation. For example, it may be necessary to impregnate the fabric with an aqueous solution of an acid or an alkali, such as citric acid, ammonium oxalate or sodium bicarbonate, and, in some cases, a reducing agent for the dye. Such materials may also be incorporated directly into the toner composition. All the aforesaid fixation procedures are well-known in the art.

After permanent fixation of the dye and/or chemical treating agent, the printed fabric is scoured to remove the ferromagnetic component, resin and any unfixed dye and/or chemical treating agent. Although the severity of the scouring treatment generally depends on the type of resin employed, with the ferromagnetic toners of this invention immersion in an aqueous surfactant solution at less than 90° C for only a few seconds usually is sufficient to dissolve away the resin and release the magnetic materials from the fabric surface. If the toner contains a dye, a well-defined colored print is obtained on the fabric.

The transfer of the ferromagnetic toner to the surface of the fabric and the temporary fixation thereof on the fabric are carried out sequentially, one immediately after the other. The permanent fixation and scouring may be done separately in a later operation, if desired.

It is to be understood that the aforesaid description of magnetic printing processes is not intended to be a limitation on the use of the ferromagnetic toners of this invention, but rather, it is intended merely to show at least one utility for such toners.

## EXAMPLES

In the following examples, unless otherwise noted, all parts and percentages are by weight and all materials employed are readily commercially available.

### EXAMPLE 1

This example illustrates the preparation, by manual mixing of the ingredients followed by spray-drying, of a ferromagnetic toner containing a blue disperse dye, magnetic components and an aqueous alkali-soluble resin, and the application thereof to both paper and polyester. A magnetic toner was prepared from 32.7% of carbonyl iron, 32.7% of  $Fe_3O_4$ , 1.8% of C.I. Disperse Blue 56, 5.5% of ligninsulfonate dispersant and 27.3% of a polyvinyl acetate copolymer resin. The carbonyl iron, used as the soft magnetic material and commercially available under the trade name "Carbonyl Iron" GS-6, is substantially pure iron powder produced by the pyrolysis of iron carbonyl. A suitable  $Fe_3O_4$  is sold under the trade name "Mapico" Black Iron Oxide and the polyvinyl acetate copolymer resin, under the trade name "Gelva" C5-VIOM. "Gelva" C5-VIOM is an aqueous alkali-soluble copolymer of vinyl acetate and a monomer containing the requisite number of carboxy groups and has a softening point of 123° C.

A 20% aqueous alkaline solution (450 parts) of the polyvinyl acetate copolymer resin was manually stirred with 500 parts of water until thorough mixing was effected. Carbonyl Iron GS-6 (108 parts) and "Mapico" Black Iron Oxide (108 parts) were added and the mixture was thoroughly stirred. C.I. Disperse Blue 56 (24

parts of a 24.6% standardized powder) was stirred in 455 parts of water until completely dispersed, then added to the above resin solution. The resultant toner slurry was stirred for 30 minutes with a high shear mixer and then spray-dried in a Niro electric spray-dryer. The toner slurry was atomized by dropping it onto a disc rotating at 20,000 to 50,000 rpm in a chamber through which heated air was swirling at a high velocity. Precautions were taken to stir the toner slurry and maintain a uniform feed composition. The exact 10 temperature and air velocity depend mainly on the softening point of the resin. An air inlet temperature of 225° C, an outlet temperature of 85° C and an atomizer air pressure of 85 psig (6 kg per sq cm gauge) provided satisfactory results. The resulting discrete toner particles of magnetic resin-encapsulated dye had a particle size within the range of 2 to 100 microns, mostly within the range of 10 to 25 microns. The particles were collected in a collection chamber. Toner adhering to the 15 sides of the drying chamber was removed by brushing into a bottle and combined with the initial fraction. The toner sample was finally passed through a 200 mesh screen (U.S. Sieve Series), thus being less than 74 microns in particle size. The ferromagnetic toner was mechanically mixed with 0.2% of a fumed silicate, Quso 20 WR-82, to improve powder flow characteristics.

Toner evaluation was made on a 2 mil (0.0508 mm) aluminized "Mylar" polyester film continuously coated with 170 microinches (43,180 Å) of acicular CrO<sub>2</sub> in a resin binder. Suitable acicular CrO<sub>2</sub> can be prepared by well known prior art techniques. The CrO<sub>2</sub> film was magnetically structured to 300 lines per inch (12 per mm) by recording a sine wave with a magnetic write head. A film positive of the printed image to be copied was placed in contact with the magnetically structured CrO<sub>2</sub>-coated aluminized polyester film and uniformly illuminated by a Xenon flash passing through the film positive. The dark areas of the film positive corresponding to the printed message absorbed the energy of the Xenon flash, whereas the clear areas transmitted the light and heated the CrO<sub>2</sub> beyond its 116° C Curie point, thereby demagnetizing the exposed magnetic CrO<sub>2</sub> lines. The latent magnetic image was manually decorated by pouring the fluidized toner powder over the 30 partially demagnetized CrO<sub>2</sub> film and then blowing off the excess. The magnetic image became visible by virtue of the toner being magnetically attracted to the magnetized areas.

The toner decorated image was separately transferred to paper and to polyester fabric substrates by applying a 20 KV positive potential from the backside of the substrate by means of a DC corona. The applied potential induced a dipole in the toner and the toner was electrostatically transferred to the substrate. Other transfer means can also be employed, such as by means of a pressure of 20-400 pounds per linear inch (0.36-7.15 kg per linear mm). However, such means may lead to shorter film life, poorer transfer efficiency and poorer image definition on the substrate. After transfer to the paper or fabric substrate, the toner was fused thereon by infrared radiation, backside fusion (140° C) or by steam fusion (100° C for 10-15 seconds at 1 atm pressure). The latter method is the most economical but is only possible with water-soluble resins.

The image which had been transferred to the paper was then heat transfer printed from the paper to polyester fabric by placing the fused image-bearing paper face-down on the polyester and applying 1.5 to 2.0 psi

5

(0.11 to 0.14 kg per sq cm) pressure for 30 seconds at 205-210° C. After direct transfer and fusion to polyester fabric, the dye was fixed in the fabric by heating for 30 seconds at 205°-210° C and 1.5 to 2.0 psi pressure (0.11 to 0.14 kg per sq cm).

Both fabric samples which had been printed as described above, that is, either directly printed or heat transfer printed from paper, following fixation of the dye, were scoured by immersion in cold water and then in hot detergent. A detergent consisting of sodium phosphates, sodium carbonates and biodegradable anionic and nonionic surfactants ("Lakeseal") was used. The samples were finally rinsed in cold water and dried. A deep blue print was obtained on each fabric.

15

#### EXAMPLE 2

This example illustrates the preparation, by ball-milling of the ingredients followed by spray-drying, of a ferromagnetic toner containing a blue disperse dye, magnetic components and an aqueous alkali-soluble resin, and the application thereof to polyester. A magnetic toner was prepared from 30% of carbonyl iron, 30% of Fe<sub>3</sub>O<sub>4</sub>, 10% of C.I. Disperse Blue 56 and 30% of a polyvinyl acetate copolymer resin ("Gelva" C5-20 VION).

A mixture of 300 parts of a 20% aqueous alkaline solution of the polyvinyl acetate copolymer resin, 20 parts of C.I. Disperse Blue 56 crude powder, 60 parts of "Mapico" Black Iron Oxide, 60 parts of Carbonyl Iron GS-6 and 100 parts of water was ball-milled for 17 hours at 37% nonvolatiles. A ceramic ball-mill was selected of such size that when the ball-mill was about one-half to two-thirds full of 0.5 inch (1.27 cm) high density ceramic balls, the above ingredients just covered the balls. After discharging the ball-mill and diluting with 460 parts of water to reduce the total nonvolatile solids to approximately 20%, the slurry was spray-dried in a Niro spray-dryer using an air inlet temperature of 200° C, an air outlet temperature of 80° C and an atomizer air pressure of 80 psig (5.6 kg per sq cm gauge). The toner particles were brushed from the drying chamber, collected and passed through a 200 mesh screen. The toner sample was fluidized with 0.2% of Quso WR-82 and then used to decorate the latent magnetic image on a 300 line per inch (12 per mm) CrO<sub>2</sub> coated aluminized "Mylar" film as described in Example b 1. The toner decorated image was electrostatically transferred directly to 100% polyester double-knit fabric by applying a 20 KV negative potential to the backside of the fabric. The toner was steam fused to the fabric at 100° C for 10-15 seconds at 1 atm pressure. After fusion, the dye was fixed in the fabric by heating at 205° C for 40 seconds at 1.5 psi (0.11 kg per sq cm). The printed fabric was then scoured at 65° C in a mixture of 2 parts per liter of caustic soda, 2 parts per liter of sodium hydrosulfite and 2 parts per liter of a polyoxyethylated tridecanol surface-active agent to remove resin, Fe, Fe<sub>3</sub>O<sub>4</sub> and any unfixed dye and then dried. A bright blue print was obtained.

35

40

45

50

55

60

65

#### EXAMPLE 3

This example illustrates the preparation of a solvent ball-milled and spray-dried, ferromagnetic resin encapsulated, disperse dye toner and the application thereof to polyester.

A magnetic toner was prepared by ball-milling a mixture of 120 parts of an aqueous alkali-soluble polyamide resin-dicarboxylic acid adduct (commercially

obtained; it exhibited superior tinctorial strength as compared to a corresponding print which had not been sprayed prior to fixation.

#### EXAMPLE 35

This example illustrates the effect of various chemicals which are normally used in the conventional printing of nylon to prevent side effects during fixation of the dye.

The toner of Example 27 containing 2% of benzalide carrier was directly printed on "Qiana" nylon fabric according to the procedure of Example 1. The toner was steam fused at 100° C and 1 atm pressure for 10-15 seconds. The fabric was then sprayed with a solution of 100 parts of urea, 10 parts of sodium chlorate and 10 parts of citric acid in 1,000 parts of water and the dye was fixed by high pressure steaming at 22 psig (1.55 kg per sq cm gauge) for 1 hour. After scouring, a deep red print was obtained; it was tinctorially stronger than a corresponding red print which had not been sprayed prior to fixation.

#### EXAMPLE 36

This example illustrates the preparation and application of a ferromagnetic disperse dye toner to a polyester/cotton blend fabric.

A 6-inch (15 cm) wide, 3-yard (274 cm) length of 65/35 polyester/cotton blend fabric was pretreated by padding to about 55% pickup with an aqueous solution containing 120 parts per liter of methoxypolyethylene glycol, M.W. 350. The padded fabric was heated at 72° C for 1 hour in a hot air oven to evaporate water, leaving the cotton fibers in a swollen state.

A magnetic toner was prepared by spray-drying a mixture containing 29.4% of polyvinyl acetate copolymer resin ("Gelva" C5-VIOM), 33.3% of Carbonyl Iron GS-6, 33.3% of "Mapico" Black Iron Oxide, 2% of a dye of the formula shown as (A) in Table VII and 2% of a sulfonated naphthalene-formaldehyde dispersant. The spray-dried product was sieved through a 200 mesh screen and 0.2% of Quso WR-82 was added to render the toner free flowing.

A latent magnetic image such as described in Example 1 was manually decorated with the above toner and transferred electrostatically to both untreated and pre-treated 65/35 polyester/cotton by a procedure such as described in Example 1. Following transfer, the toner was steam fused at 100° C and 1 atm pressure for 10 to 15 seconds and the dye was hot air fixed at 205° C for 100 seconds. Following fixation of the dye, the print was scoured at 65° C in aqueous detergent. The pre-treated polyester/cotton fabric was printed in a deep bright red shade, whereas the untreated fabric was only lightly stained. Similar results were obtained when the disperse dye toner was transferred to the pretreated and untreated fabrics, steam fused and then dry heat fixed at 205° C for 100 seconds at 1.5 psig (0.11 kg per sq cm gauge).

#### EXAMPLE 37

This example illustrates the preparation of a ferromagnetic toner containing a cationic dye, magnetic components and an aqueous alkali-soluble resin and the application thereof to acid-modified polyester and polyacrylonitrile.

A solution of 21 parts of C.I. Basic Blue 77, as a 24.4% standardized powder (containing boric acid as a diluent) in 300 ml of hot water, was added, with thor-

ough stirring, to 400 parts of a 20% aqueous alkaline solution of a polyvinyl acetate resin ("Gelva" C5- VIOM). Carbonyl Iron GS-6 (91 parts), "Mapico" Black Iron Oxide (91 parts) and 510 parts of water were then added and stirring was continued for an additional 30 minutes. The toner slurry was spray-dried to give a final toner composition containing 28.3% of polyvinyl acetate copolymer resin, 32.2% of Carbonyl Iron GS-6, 32.2% of "Mapico" Black Iron Oxide, 1.8% of C.I. Basic Blue 77 and 5.5 weight percent of boric acid diluent. The toner was sieved through a 200 mesh screen and fluidized with 0.2% of Quso WR-82.

A latent magnetic image such as described in Example 1 was manually decorated with the above toner and transferred electrostatically to acid-modified polyester fabric as described in Example 1. After transfer, the toner was steam fused at 100° C and 1 atm pressure for 10 to 15 seconds and the cationic dye was fixed by high-pressure steaming at 22 psig (1.55 kg per sq cm gauge) for 1 hour. The printed fabric was scoured as described in Example 2. A blue print was obtained.

A second toner transfer was made to polyacrylonitrile fabric in a similar manner. The toner was steam fused, the dye was fixed by cottage-steaming at 7 psig (0.5 kg per sq cm gauge) for 1 hour and the printed fabric was scoured as described above; a deep blue print was obtained.

In conventional printing with cationic dyes, a "steady acid" is normally used in the print paste to insure that an acid pH is maintained during fixation of the dye. Accordingly, in another set of experiments, after transfer and steam fusion of the above cationic dye toner to both the acid-modified polyester and the polyacrylonitrile fabrics, the printed fabrics were oversprayed with a 50% aqueous solution of citric acid and then fixed by high-pressure steaming and cottage-steaming, respectively, as described above. The printed fabrics were then scoured. Bright blue prints were obtained, exhibiting superior image definition as compared to the prints which were prepared without the overspray step.

#### EXAMPLES 38 TO 43

Ferromagnetic cationic dye toners were prepared by manually mixing the appropriate ingredients and spray-drying the slurries as described in Example 37. After drying, 0.2 to 1.2% of Quso WR-82 was added to obtain toner fluidity. Details are summarized in Table II. The ferromagnetic cationic dye toners were directly printed to both acid-modified polyester and polyacrylonitrile substrates, steam fused and fixed by either high pressure steam development at 22 psig (1.55 kg per sq cm gauge) for 1 hour or by cottage-steaming at 7 psig (0.5 kg per sq cm gauge) for 1 hour.

Cationic dyes of the triarylmethane (Example 37), azomethine (Example 38), styryl (Examples 39 and 41-43) and rhodamine (Example 40) series, with both water-soluble hydroxypropyl cellulose ("Klucel" LF) and polyvinyl acetate copolymer ("Gelva" C5- VIOM) resins, are exemplified. "Klucel" LF is a cellulose ether containing propylene glycol groups attached by an ether linkage and not more than 4.6 hydroxypropyl groups per anhydroglucose unit and having a molecular weight of approximately 100,000. The cationic dye toners of Examples 42 and 43 containing 1 and 2%, respectively, of citric acid provided brighter and tinctorially stronger prints on both acid-modified polyester and polyacrylonitrile as compared to the corresponding toners without the citric acid.

available as TPX-1002), 136 parts of "Mapico" Black Iron Oxide, 136 parts of Carbonyl Iron GS-6, 8 parts of C.I. Disperse Red 60 crude powder and 267 parts of a 50:50 mixture of toluene:isopropanol for 16 hours at 60% nonvolatile solids. The ball-mill was discharged and the contents was diluted with 666 ml of a 50:50 mixture of toluene:isopropanol to approximately 30% nonvolatile solids. The solvent toner slurry was spray-dried in a Bowen spray-dryer using a feed rate of 152 ml per minute, an air inlet temperature of 143° C, an air outlet temperature of 62° C and an atomizer air pressure of 85 psig (6 kg per sq cm gauge). The toner particles were classified to some extent by a cyclone collection system. The main toner fraction (81%, 238 parts) collected from the dryer chamber consisted of nearly spherical spray-dried particles having an average particle size of 10 to 15 microns (a range of 2 to 50 microns). The resultant magnetic toner consisted of 30% of polyamide resin adduct, 34% of carbonyl iron, 34% of  $Fe_3O_4$  and 2% of C.I. Disperse Red 60. The toner was fluidized with 0.3% of Quso WR-82 and then applied to decorate the latent image on a 300 line per inch (12 per mm) magnetically structured  $CrO_2$  coated aluminized "Mylar" film as described in Example 1. The toner decorated image was electrostatically transferred directly to 100% polyester woven fabric by applying a 20 KV negative potential to the backside of the fabric. The fabric was steam fused and the dye was fixed by heating at 205° C for 40 seconds at 1.5 psi (0.11 kg per sq cm). The printed fabric was then scoured as in Example 2 and dried.

#### EXAMPLES 4 TO 33

Disperse dye toners were prepared by either manually mixing or ball-mixing the appropriate ingredients and spray-drying the slurry as described in Examples 1 and 2. Details are summarized in Table I. Manually mixed toners were prepared in all cases except Examples 13, 14, 19 and 32; in these the toners were prepared by ball-milling. The compositions of the final spray-dried toners as well as the ratio of resin to total magnetic component present are also shown in the table. Ball-milled toners exhibited optical densities, when printed on polyester, which were superior to those of manually mixed toners of comparable dye concentration. This difference is particularly evident when the toner contains high concentrations of dye. The standardized disperse dye powders (and pastes) used in the manually mixed toners contained ligninsulfonate and sulfonated naphthalene-formaldehyde condensate dispersing agents. At high dispersant levels, the quantity of magnetic component in the toner becomes limited and decoration of the latent magnetic image may become impaired.

Toner compositions containing 9 to 74% (Examples 12 and 25) of water-soluble resin and 14 to 83% (Examples 11 and 12) of total magnetic component and compositions having a resin to magnetic component ratio of 0.11 to 3.3 (Examples 12 and 25) exhibited satisfactory magnetic, transfer and fusion properties. Various disperse dye types, for example, quinophthalone (Example 4), anthraquinone (Examples 5 to 25, 32 and 33) and azo (Examples 26 to 31) dyes, provide a wide range of colored magnetic toners. The amount of dye present in the toner depends on the amount of resin and magnetic component present. Dye concentrations of 0.10% (Example 33) to 25% (Example 32) were used with satisfactory results. Toner compositions containing both hard

and soft magnetic components are exemplified in Table I. A binary mixture of magnetic particles is not essential, however, Equally good results are obtained using only a hard magnetic component (Examples 18 to 21). Ferric oxide is a preferred hard magnetic component based on its magnetic properties and its cost. Chromium dioxide can also be used but it is much more expensive. A free-flow agent, present in quantities of 0.01 to 5% (preferably 0.01 to 0.4%), based on total toner weight, was used to keep the individual toner particles from sticking together and to increase the bulk of the toner powder. These factors facilitate even deposition of toner over the imaging member. Free-flow agents such as microfine silica and alumina are useful. Quso WR-82 provides satisfactory flow properties when added to the toners described herein.

The toners were evaluated as described in Example 1. The latent magnetic image on a 300 line per inch (12 per mm) magnetically structured  $CrO_2$ -coated aluminized "Mylar" film was manually decorated and the decorated image was electrostatically transferred to (that is, printed on) a substrate (shown in Table I). The toner fusion and dye fixation conditions and the scouring procedure for removing resin, magnetic component(s) and unfixed dye from the printed substrate are also given in the table. For instance, in Example 4 the designation "DP(Pap)" indicates that the toner was directly printed on paper and infrared fused at 160°-170° C; the designation "HTP(PE)" means that the toner was heat transfer printed from paper to polyester by heating at 205° C for 40 seconds and 1.5 psi (0.11 kg per sq cm) and the printed polyester was scoured at 65° C in aqueous detergent solution; and the designation "DP(PE)" means that the toner was directly printed on polyester, infrared fused at 160°-170° C, the dye was fixed at 205° C for 40 seconds and 1.5 psi (0.11 kg per sq cm) and the printed polyester fabric was scoured at 65° C. in aqueous detergent.

A number of different fixation procedures, for example, dry heat, hot air, high temperature steam and high pressure steam, were used to fix the dyes in the substrate. Such procedures are well-known in the art for fixing disperse dyes in polyester and nylon.

Examples 27, 29, 30 and 31 show the effect of incorporating 2, 4, 6 and 8% of a benzidine dye carrier in the toner compositions. The carrier gave increased tinctorial strength over toner without the carrier. Concentrations of 2 to 4% (of carrier) provided optimum results.

#### EXAMPLE 34

This example illustrates the effect of various chemicals which are normally used in the conventional printing of polyester to prevent side effects during fixation of the dye.

The toner of Example 27 containing 2% of benzidine carrier was directly printed on 100% polyester woven fabric according to the procedure of Example 1. The toner was steam fused at 100° C and 1 atm pressure for 10-15 seconds. The fabric was sprayed with a solution of 100 parts of urea and 10 parts of sodium chlorate in 1,000 parts of water to prevent reduction of the dye during the fixation step. The dye was fixed by high pressure steaming at 22 psig (1.55 kg per sq cm gauge) for 1 hour. The printed fabric was scoured in 2 parts per liter of sodium hydrosulfite, 2 parts per liter of soda caustic and 2 parts per liter of a polyethoxylated tridecanol surfactant at 65° C. A deep red print was

## EXAMPLE 44

This example illustrates the preparation of a ferromagnetic toner containing an acid dye, magnetic components and an aqueous alkali-soluble resin and the application thereof to nylon.

A solution of 12.7 parts of C.I. Acid Blue 40 (C.I. 62,125), as a 31.6% standardized powder (containing dextrin as a diluent) in 150 ml of hot water, was added, with thorough stirring, to 300 parts of a 20% aqueous alkaline solution of a polyamide resin (TPX-1002). Carbonyl Iron GS-6 (63.4 parts), "Mapico" Black Iron Oxide (64 parts) and 410 parts of water were added and the slurry was stirred on a high shear mixer for 20 minutes. The toner slurry was spray-dried to give a final toner composition containing 30% of polyamide resin, 31.7% of Carbonyl Iron GS-6, 32% of "Mapico" Black Iron Oxide, 2% of C.I. Acid Blue 40 and 4.3% of dextrin diluent. The toner was sieved through a 200 mesh screen and fluidized with 0.6% of Quso WR-82.

A latent magnetic image such as described in Example 1 was manually decorated with the above toner and transferred electrostatically to 100% nylon 66 jersey fabric and steam fused at 100° C and 1 atm pressure for 10 to 15 seconds. The acid dye was fixed by cottage-steaming the printed fabric at 7 psig (0.5 kg per sq cm gauge) for 1 hour. The fabric was scoured at 60° C with an aqueous solution of 2 parts per liter of a polyethoxylated oleyl alcohol and 2 parts per liter of alkyl trimethylammonium bromide surface-active agents. A 30 bright blue print was obtained.

## EXAMPLES 45 TO 53

Ferromagnetic acid dye toners were prepared by manually mixing the appropriate ingredients and spray-drying the slurries as described in Example 44. The toners were fluidized with 0.2 to 1.4% of Quso WR-82. Details are summarized in Table III. A latent magnetic image such as described in Example 1 was manually decorated and the toner decorated image was electrostatically transferred directly to nylon 66 jersey. The toners were steam fused and the acid dyes were fixed by cottage-steaming at 7 psig (0.5 kg per sq cm gauge) for 1 hour. After scouring, bright well-defined prints were obtained.

Toners containing monosulfonated azo (Examples 45, 46 and 51) and monosulfonated anthraquinone (Examples 47 to 50) dyes, with water-soluble polyvinyl acetate copolymer ("Gelva" C5-VIOM), hydroxypropylcel lulose ("Klucel" LF) and polyamide (TPX-1002) resins, are exemplified. Examples 52 and 53 include a special disulfonated bis-anthraquinone dye which is noted for its good light- and wetfastness properties on nylon. Examples 47, 50, 51 and 53, with acid dyes and containing 1% of ammonium oxalate, provided brighter and tintorially stronger prints on nylon than the corresponding toners without ammonium oxalate. Citric acid, present either in the toner (Example 49) or sprayed on the toner fused nylon (Example 48), was found to significantly improve dye fixation.

## EXAMPLE 54

This example illustrates the preparation of a ferromagnetic toner containing a fiber-reactive dye, magnetic components and an aqueous alkali-soluble resin and the application thereof to cotton.

A magnetic toner was prepared by spray-drying a mixture containing 30% of polyvinyl acetate copolymer

resin ("Gelva" C5-VIOM), 33% of Carbonyl Iron GS-6, 33% of "Mapico" Black Iron Oxide, 2% of C.I. Reactive Blue 7 (C.I. 61125) and 2% of inorganic diluent. The spray-dried product was sieved through a 200 mesh screen and fluidized with 0.3% Quso WR-82. A latent magnetic image such as described in Example 1 was manually decorated with the above toner and the decorated image was electrostatically transferred to 100% cotton twill fabric by applying a 20 KV negative potential to the backside of the fabric. The printed fabric was steam fused at 100° C and 1 atm pressure for 10 seconds. The toner fused cotton fabric was then sprayed with an aqueous solution containing 100 parts per liter of urea and 15 parts per liter of sodium bicarbonate. This overspray is required to chemically link the reactive dye to the cotton by forming a covalent dye-fiber bond. Following the spray application, the cotton fabric was dried and the dye was fixed by heating at 190° C for 3 minutes in a hot air oven. The fabric was then scoured at 65° C in aqueous detergent. A brilliant blue print having excellent washfastness properties was obtained.

## EXAMPLE 55

A spray-dried magnetic toner containing 30% of polyvinyl acetate copolymer resin ("Gelva" C5- VIOM), 33% of Carbonyl Iron GS-6, 33% of "Mapico" Black Iron Oxide, 2% of Reactive Yellow 2 and 2% of inorganic diluent was directly printed on 100% cotton twill fabric in general accord with the procedure described in Example 54. The toner was steam fused and the printed fabric was sprayed with an aqueous solution containing 100 parts per liter of urea and 15 parts per liter of sodium bicarbonate. The dye was fixed by heating at 182° C for 3 minutes and the fabric was scoured at 65° C in aqueous detergent. A bright yellow print was obtained.

## EXAMPLE 56

Following the procedure of Example 55, a spray-dried ferromagnetic toner containing 30% of polyvinyl acetate copolymer resin ("Gelva" C5- VIOM), 33% of Carbonyl Iron GS-6, 33% of "Mapico" Black Iron Oxide, 2% C.I. Reactive Red 2 and 2% of diluent was directly printed on 100% cotton twill fabric. The toner was steam fused, the printed fabric was oversprayed with aqueous urea/sodium bicarbonate and the dye was fixed. After scouring, a bright red print was obtained.

## EXAMPLE 57

This example illustrates the preparation of a ferromagnetic toner containing a reactive dye, a disperse dye, magnetic components and an aqueous alkali-soluble resin and the application thereof to polyester/cotton-blend fabric.

A magnetic toner was prepared by spray-drying a mixture containing 30% of polyvinyl acetate copolymer resin ("Gelva" C5- VIOM), 30% of Carbonyl Iron GS-6, 31.1% of "Mapico" Black Iron Oxide, 3% of a 60/40 mixture of a yellow disperse dye of the formula shown as (B) in Table VII and C.I. Reactive Yellow 2 and 5.9% of inorganic diluent. The toner was sieved through a 200 mesh screen and fluidized with 0.2% of Quso WR-82. Toner decoration of a latent magnetic image was carried out as described in Example 1. The toner decorated image was electrostatically transferred directly to 65/35 polyester/cotton poplin fabric and steam fused at 100° C and 1 atm pressure for 10 seconds. Dye fixation was accomplished by heating the fabric at

210° C for 100 seconds in a hot air oven. The printed fabric was finally scoured at 60° C in aqueous detergent. A bright yellow well-defined print was obtained.

#### EXAMPLE 58

A spray-dried magnetic toner containing 30% of polyvinyl acetate copolymer resin ("Gelva" C5- VIOM), 30% of Carbonyl Iron GS-6, 30.1% of "Mapico" Black Iron Oxide, 3% of a 76/24 mixture of a blue disperse dye of the formula shown as (C) in Table VII and C.I. Reactive Blue 7 and 6.9% of inorganic diluent was directly printed on 65/35 polyester/cotton poplin and steam fused as described in Example 57. The printed fabric was fixed by heating at 200° C for 100 seconds and then scoured at 60° C in aqueous detergent. 15 A bright blue print was obtained.

#### EXAMPLE 59

This example illustrates the preparation of a ferromagnetic toner containing a sulfur dye, magnetic components and an aqueous alkali-soluble resin and the application thereof to cotton.

A spray-dried magnetic toner containing 32.6% of polyvinyl acetate copolymer resin ("Gelva" C5- VIOM), 32.6% of Carbonyl Iron GS-6, 32.6% of 25 "Mapico" Black Iron Oxide and 2.2% of C.I. Leuco Sulfur Blue 13 (C.I. 53450) was prepared, sieved through a 200 mesh screen and fluidized with 0.2% of Quso WR-82. A toner decorated latent magnetic image was electrostatically transferred, by a procedure such as 30 described in Example 1, to 100% cotton fabric. The toner was steam fused at 100° C and 1 atm pressure for 10 seconds. The printed fabric was subsequently padded from an aqueous bath containing 300 parts per liter of sodium sulfhydrate at a pickup of approximately 50%. The leuco dye was then immediately steam fixed at 100° 35 C and 1 atm pressure for 60 seconds. After fixation, the printed fabric was developed by oxidation at 50° C in an aqueous bath containing 4 parts per liter of sodium perborate. The fabric was finally scoured at 60° C in an aqueous bath containing 2 parts per liter of diethanolamine oleyl sulfate surface-active agent. A blue print 40 was obtained.

#### EXAMPLE 60

This example illustrates the preparation of a ferromagnetic toner containing a vat dye, magnetic components and an aqueous alkali-soluble resin and the application thereof to cotton fabric.

A spray-dried magnetic toner containing 29% of 50 polyvinyl acetate copolymer resin ("Gelva" C5- VIOM), 32.9% of Carbonyl Iron GS-6, 32.9% of "Mapico" Black Iron Oxide, 2.7% of C.I. Vat Red 10 (C.I. 67,000) and 2.5% of diluent was used to manually 55 decorate a latent magnetic image on a 300 line per inch (12 per mm) magnetically structured CrO<sub>2</sub> coated aluminized "Mylar" film. The toner decorated latent image was electrostatically transferred to 100% cotton twill fabric and the toner was steam fused at 100° C and 1 atm pressure for 10 seconds. The printed cotton fabric was 60 then padded from a reducing bath containing

30 parts per liter of soda caustic

60 parts per liter of soda ash

60 parts per liter of sodium hydrosulfite

2 parts per liter of sodium octyl/decyl sulfate surface- 65 active agent

15 parts per liter of amylopectin thickening agent

2 parts per liter of 2-ethylhexanol

at a pickup of 70 to 80% and flash aged at 132° C for 45 seconds. The fabric was rinsed in cold water, oxidized for 1 minute at 60° C in a bath containing 2% hydrogen peroxide and 2% glacial acetic acid, rinsed and scoured for 5 minutes at 82° C in 0.5 part per liter (aqueous) of a diethanolamine oleyl sulfate surface-active agent. A bright red print was obtained.

#### EXAMPLE 61

10 A spray-dried ferromagnetic toner containing 30% of polyvinyl acetate copolymer resin ("Gelva" C5- VIOM), 33% of Carbonyl Iron GS-6, 33% of "Mapico" Black Iron Oxide, 2% of C.I. Vat Blue 6 (C.I. 69825) and 2% of diluent was prepared and the latent image produced therewith was transferred directly to 100% cotton twill fabric. The toner was fused, the vat dye was fixed and the printed fabric was scoured as described in Example 60. A bright blue print was obtained.

#### EXAMPLE 62

A spray-dried ferromagnetic toner containing 30% of polyvinyl acetate copolymer resin ("Gelva" C5- VIOM), 33% of Carbonyl Iron GS-6, 33% of "Mapico" Black Iron Oxide, 2% of C.I. Vat Yellow 22 and 2% of diluent was prepared and printed on 100% cotton twill fabric by a procedure substantially as described in Example 60. A yellow print was obtained.

#### EXAMPLE 63

This example illustrates the preparation of a ferromagnetic toner containing a premetallized acid dye, magnetic components and an aqueous alkali-soluble resin and the application thereof to nylon.

A spray-dried magnetic toner was prepared so as to contain 30% of polyvinyl acetate copolymer resin ("Gelva" C5- VIOM), 31.4% of Carbonyl Iron GS-6, 31.4% of "Mapico" Black Iron Oxide, 2% of C.I. Acid Yellow 151 (a sulfonated premetallized azo dye) and 5.2% of inorganic diluent. The toner was sieved through a 200 mesh screen and fluidized with 0.2% of Quso WR-82. A toner decorated latent magnetic image such as described in Example 1 was electrostatically transferred to nylon 66 jersey fabric and steam fused at 100° C and 1 atm pressure for 10 seconds. The premetallized acid dye was fixed by cottage-steaming the fabric at 7 psig (0.5 kg per sq cm gauge) for 1 hour. The printed fabric was then scoured at 65° C in an aqueous solution of 2 parts per liter of each of sodium hydrosulfite, soda caustic and polyethoxylated tridecanol surfactant. A second toner transfer was made to nylon 66 jersey fabric. The toner was steam fused and the fabric was oversprayed with a 50% aqueous solution of citric acid. The dye was fixed by cottage-steaming at 7 psig (0.5 kg per sq cm gauge) for 1 hour and the printed fabric was caustic-hydro scoured as above. In both cases, strong well-defined yellow prints were obtained.

#### EXAMPLE 64

Using the procedures substantially as disclosed in Example 63, a spray-dried ferromagnetic toner containing 30% of polyvinyl acetate copolymer resin ("Gelva" C5- VIOM), 32.1% of Carbonyl Iron GS-6, 33% of "Mapico" Black Iron Oxide, 2% of C.I. Acid Red 182 (premetallized azo dye) and 2.9% of inorganic diluent was prepared and electrostatically transferred to nylon 66 jersey fabric. After steam fusing, cottage-steaming and scouring, a well-defined bright red print fabric was obtained. A similar sharp red print was obtained when

the fabric was oversprayed with 50% aqueous citric acid prior to cottage-steaming.

#### EXAMPLES 65 to 68

Examples 65 to 68 illustrate the preparation of ferromagnetic toners containing cationic-disperse dyes, magnetic components and an aqueous alkali-soluble resin and the application thereof to acid-modified polyester, polyacrylonitrile and cellulose acetate.

Cationic-disperse dyes, that is, water-insoluble salts of dye cations and selected arylsulfonate anions, are well-known in the art for dyeing acid-modified polyester and acrylic fibers. Cationic-disperse dye toners were prepared by manually mixing the appropriate ingredients (20% nonvolatile solids) and spray-drying. The 15 spray-dried toners were sieved through a 200 mesh screen and fluidized with 0.2% of Quso WR-82. Details are summarized in Table IV. Examples 65 to 67 use 1,5-naphthalenedisulfonate as the anion and Example 68 uses 2,4-dinitrobenzenesulfonate as the anion. Toner 20 decoration of a latent magnetic image and electrostatic transfer to the fabric substrate were preformed as described in Example 1. The toners were steam fused and the printed fabrics were oversprayed with 50% aqueous citric acid to aid in dye fixation. The dyes were fixed by 25 either cottage-steaming or high-pressure steaming the sprayed fabrics. After scouring, in each example, a well-defined print was obtained.

#### EXAMPLE 69

This example illustrates the preparation of a ferromagnetic toner containing a fluorescent brightening agent, magnetic components and an aqueous alkali-soluble resin and the application thereof to cotton.

A magnetic toner containing 30% of polyvinyl acetate copolymer resin ("Gelva" C5-VIOM), 34% of Carbonyl Iron GS-6, 34% of "Mapico" Black Iron Oxide and 2% of C.I. Fluorescent Brightener 102 was prepared by spray-drying an aqueous 20% nonvolatile solids mixture of the ingredients. The spray-dried toner was sieved through a 200 mesh screen and fluidized with 0.2% of Quso WR-82. A latent magnetic image such as described in Example 1 was toner decorated and the image was electrostatically transferred to 100% cotton sheeting. The toner was steam fused and the 45 brightener was fixed by heating the fabric at 100°C and 1 atm pressure for 25 minutes. The printed fabric was then scoured at 60°C in an aqueous solution of 2 parts per liter of soda caustic and 2 parts per liter of polyethoxylated tridecanol surfactant. Upon exposure to an ultraviolet light source, the printed fabric strongly fluoresced in the image areas.

#### EXAMPLES 70 to 74

These examples illustrate the preparation of ferromagnetic toners containing a chemical-resist agent, magnetic components and an aqueous alkali-soluble resin and the application thereof to nylon. The toners were prepared by spray-drying an aqueous 20% nonvolatile solids slurry of the appropriate ingredients. The 55 spray-dried toners were sieved through a 200 mesh screen and fluidized with 0.2% of Quso WR-82. Details are summarized in Table V. The chemical-resist toners were evaluated by manual decoration of the latent magnetic image on a 300 line per inch (12 per mm) magnetically structured CrO<sub>2</sub>-coated aluminized "Mylar" film by procedures substantially the same as described in Example 1. The toner-decorated images were trans-

ferred electrostatically to nylon 66 jersey fabric and steam fused at 100°C and 1 atm pressure for 10 to 15 seconds. The chemical resist in each example was fixed by steaming (atmospheric) the fabric for 20 minutes.

5 Each printed fabric was rinsed in water to remove the resin and the magnetic component(s) and finally dried. Each resultant resist printed nylon fabric was then overdye with either a red biscationic dye of the formula shown as (D) or a blue diacidic (anionic) dye of the formula shown as (E), or a mixture thereof, the (D) and (E) formulas being given in Table VII, by the following procedure:

Resist-printed nylon fabric (5 parts) was added to 300 parts of water containing:

|                                                         |                         |
|---------------------------------------------------------|-------------------------|
| ethylenediaminetetraacetic acid, tetrasodium salt       | 0.013 part (0.25% o/wf) |
| a sulfobetaine of the formula shown as (F) in Table VII | 0.05 part (1.0% o/wf)   |
| tetrasodium pyrophosphate                               | 0.010 part (0.2% o/wf). |

The dye bath was adjusted to pH 6 with monosodium phosphate and the temperature was raised to 27°C and held at this temperature for 10 minutes. The cationic dye (0.025 part; 0.5% o/wf, that is, on weight of fiber) and/or the acidic dye (0.025 part; 0.5% o/wf) were added. When both types of dyes were employed, the bath containing the cationic dye was held at 27°C for 5 minutes prior to the addition of the anionic dye. After completion of the dye(s) addition the bath was maintained at 27°C for 10 minutes, the temperature was raised at about 2°C per minute to 100°C and held at this temperature for 1 hour. Each fabric was rinsed in cold water and dried. The printed-resist fabrics remained unstained in the imaged areas during the subsequent overdyeing process.

30 Toners containing 2, 4, 6 and 8% of a chemical-resist agent of the formula shown as (G) in Table VII and binary soft (Fe) and hard (Fe<sub>3</sub>O<sub>4</sub>) magnetic materials are 35 illustrated in Examples 70 to 73; they showed excellent chemical-resist properties on nylon. An analogous magnetic-resist toner containing only chromium dioxide as the hard magnetic component (Example 74) also provided satisfactory printed resist on nylon.

#### EXAMPLE 75

This example illustrates the multicolor printing of polyester with ferromagnetic disperse dye toners containing water-soluble resins.

A semitransparent nonconductive CrO<sub>2</sub> film was prepared by embossing a 5-mil (0.127 mm) thick flexible cellulose acetate film with a 500 line per inch (20 per mm) pattern of parallel grooves. Chromium dioxide mixed in an alkyd binder was doctoried over the surface of the embossed transparent support and then cured to bind the magnetic material to the support by a procedure known in the art, for example, as described in U.S. Pat. No. 3,544,798. The film was magnetized by passing it over the poles of a bar magnet of approximately 1,500 gauss average field strength. A photicolor separation of a printed design was made by photographing the design three times through red, green and blue filters. Exposure through the red filter produced a negative recording of the red light in the printed original. A cyan film positive recording the remaining green and blue primaries present in the original print was obtained. Exposure through the green filter produced a negative recording

of the green in the original print, and a magenta film positive recording the remaining red and blue primaries was obtained. Similarly, exposure through the blue filter produced a negative recording of the blue in the original print, and a yellow film positive was obtained. A separate latent magnetic image of each of the cyan, magenta and yellow colors making up the design to be printed was developed by placing the photocolor separated film positive of the desired color in contact with the aforesaid magnetized semitransparent  $\text{CrO}_2$  film and uniformly illuminating by a Xenon flash passing through the film positive. The dark areas of the film positive, that is, the image areas, absorbed the energy of the Xenon flash, whereas the clear areas transmitted the light and heated the  $\text{CrO}_2$  beyond its  $116^\circ\text{C}$  Curie point, thereby demagnetizing the exposed magnetic  $\text{CrO}_2$  lines. A latent magnetic image corresponding to the dark areas of the film positive was obtained. The resultant cyan, magenta and yellow latent magnetic images were manually decorated with the blue, red and yellow disperse dye toners of Examples 1, 15 and 4, respectively. An AC corona was passed over the surface of each toner decorated image to dissipate any static charges. The cyan toner-decorated latent image was electrostatically transferred at 20 KV negative potential directly to 100% polyester woven cloth. The magenta and yellow toner-decorated images were similarly successively transferred to the same polyester fabric, thereby providing a multicolored printed design. Following transfer, the disperse dyes were fixed by heating the printed fabric at  $205^\circ\text{C}$  and 1.5 psi (0.11 kg per sq cm) for 40 seconds. The printed fabric was then scoured at  $60^\circ\text{C}$  in an aqueous solution of 2 parts per liter of sodium hydrosulfite and 2 parts per liter of soda caustic. A well-defined multicolored printed design was obtained.

#### EXAMPLE 76

A ferromagnetic disperse dye toner containing 30% of a polyamide resin ("Versamid" 930), 34% of Carbonyl Iron GS-6, 34% of "Mapico" Black Iron Oxide and 2% of C.I. Disperse Yellow 54 was prepared by ball-milling and spray-drying a 20% nonvolatile solids toluene-isopropanol slurry of the ingredients by a procedure substantially as described in Example 3. "Versamid" 930 is a water-insoluble resin having a molecular weight of about 3,100 and a softening temperature of  $105^\circ\text{--}115^\circ\text{C}$ . Such water-insoluble resins are disclosed as having utility in prior art, known magnetic toners, for example, such as disclosed by Hall and Young in U.S. Pat. No. 3,627,682.

A magnetic disperse dye toner containing 31.1% of polyvinyl acetate copolymer resin ("Gelva" C5-IVOM), 30.7% of Carbonyl Iron GS-6, 30.7% of "Mapico" Black Iron Oxide, 1.9% of C.I. Disperse Blue 56 and 5.6% of dispersant was prepared by spray-drying an aqueous slurry of the ingredients containing 20% of nonvolatile solids.

Both of the aforesaid toners were manually applied to the latent images on a  $\text{CrO}_2$ -coated aluminized "Mylar" film and electrostatically transferred to 100% polyester double-knit fabric by procedures substantially the same as described in Example 1. The toners were steam fused and the disperse dyes were fixed by heating the printed fabrics at  $210^\circ\text{C}$  and 1 atm pressure for 15 seconds. The printed fabrics were then scoured at  $75^\circ\text{C}$  in an aqueous solution of 4 parts per liter of caustic soda, 4 parts per liter of sodium hydrosulfite and 2 parts per liter of

"Lakeseal" detergent. The fabric printed with the disperse dye toner containing the water-soluble resin was completely clear of resin and magnetic components after just a few seconds of gentle stirring in the scouring medium. The fabric printed with the water-insoluble resin was not clear of resin and magnetic components even after 15 minutes scouring at  $75^\circ\text{C}$ . Thus, the resin impregnated magnetic particles were much more easily removed from the printed fabric using the dye toner containing the water-soluble resin as compared to the toner containing the water-insoluble resin. This is a critical feature since the presence of the black iron-iron oxide on the fabric surface effectively masks the color of the dye fixed in the fabric. In the aforesaid experiment employing the water-soluble polyvinyl acetate resin, scoured fabric was printed to a bright blue whereas in the experiment employing the water-insoluble polyamide resin, the scoured fabric was printed to a dark brown to black, completely masking the bright yellow color of the dye employed.

#### EXAMPLE 77

This example illustrates the preparation of a ferromagnetic dye toner containing a yellow disperse dye, magnetic components and a water-soluble natural resin, and the application thereof to paper and polyester.

A mixture of 350 parts of a commercially available 20% aqueous solution of a maleic anhydride-rosin derivative ("Unirez" 7057), 28.4 parts of C.I. Disperse Yellow 54 as a 28.2% standardized powder containing a 50/50 mixture of lignin sulfonate and sulfonated naphthalene-formaldehyde as a dispersant, 60 parts of "Mapico" Black Iron Oxide and 59.6 parts of Carbonyl Iron GS-6 was stirred for 30 minutes on a high-speed shear mixer. Water (502 parts) was added and the resultant slurry was spray-dried to give a final toner composition containing 35% of esterified rosin, 4% of C.I. Disperse Yellow 54, 1.2% of the lignin sulfonate/sulfonated naphthalene-formaldehyde dispersant, 30% of "Mapico" Black Iron Oxide and 29.8% of Carbonyl Iron GS-6. The toner was sieved through a 200 mesh (U.S. Sieve Series) screen and fluidized with 2% of Quso WR-82. A latent magnetic image such as described in Example 1 was manually decorated with the toner and the toner decorated image was transferred electrostatically to both paper and polyester substrates by applying a 20 KV negative potential, using a DC corona, to the backside of the substrate. After transfer the image was steam-fused on each substrate. After direct transfer and fusion to the polyester fabric, the dye image was fixed by heating for 30 seconds at  $210^\circ\text{C}$  and 1 to 1.5 psi (0.07 to 0.11 kg per sq cm) pressure. The dye was also heat transfer printed from the paper to polyester fabric by placing the fused image-bearing paper face down on the polyester and applying 1 to 1.5 psi (0.07 to 0.11 kg per sq cm) pressure for 30 seconds at  $210^\circ\text{C}$ . Each of the fabrics, after dye fixation, was scoured with hot aqueous alkaline detergent. Deep yellow prints were obtained on each, that is, the polyester which was directly printed and the polyester which was heat transfer printed from paper.

#### EXAMPLE 78

This example illustrates the preparation of a ferromagnetic dye toner containing a yellow disperse dye, magnetic components and an aqueous alkali-soluble polyacrylic acid resin, and the application thereof to paper and polyester.

A ferromagnetic toner was prepared by spray-drying a mixture containing 35% of a commercially available, aqueous alkali-soluble polyacrylic acid resin ("Joncryl" 678), 4% of C.I. Disperse Yellow 54, 1.2% of a 50/50 mixture of lignin sulfonate and sulfonated naphthaleneformaldehyde dispersant, 30% of "Mapico" Black Iron Oxide and 29.8% of Carbonyl Iron GS-6. The spray-dried toner was sieved through a 200 mesh (U.S. Sieve Series) screen and fluidized with 0.1% of Quso WR-82. The toner was used to manually decorate a latent magnetic image on the surface of a printing base such as described in Example 1. The decorated image was then electrostatically transferred and steam fuser to paper and subsequently heat transfer printed from the paper to 100% polyester fabric as described in Example 15. The image was also directly printed to 100% polyester fabric as described in Example 77. In both cases the fixed printed fabrics were scoured at 65° C in an aqueous polyethoxylated tridecanol surfactant solution; deep yellow prints were obtained on both fabrics.

## EXAMPLE 79

This example illustrates the preparation of a ferromagnetic dye toner containing a red disperse dye, a magnetically hard component and an aqueous alkali-soluble polyvinyl acetate copolymer resin, and the application thereof to paper and polyester film and fabric.

A ferromagnetic toner was prepared by spray-drying a mixture containing 30% of polyvinyl acetate copolymer resin, 65.8% of a commercially available  $Fe_3O_4$ -cobalt alloy ("HiEN"-527) containing 1 to 2 mole percent of cobalt, 1% of C.I. Disperse Red 60 and 3.2% of a lignin sulfonate dispersant. The toner was passed through a 200 mesh screen. The toner flow properties were excellent. The toner was used to manually decorate a latent magnetic image on the surface of a printing base such as described in Example 1. The decorated image was electrostatically transferred to paper, steam fused and then heat transfer printed from the paper to 100% of polyester fabric. The image was also directly transferred to both 100% polyester fabric and "Mylar" polyester film and then steam fused. The image was also electrostatically transferred to paper, steam fused and

then heat transfer printed from the paper. In each case permanent dye fixation was achieved by heating the printed film or fabric substrate at 205°-210° C and 1.5 psi (0.11 kg per sq cm) pressure for 40 seconds. The printed substrates were finally scoured at 82° C in an aqueous solution of 2 parts/liter of caustic soda, 2 parts/liter of hydrosulfite and 2 parts/liter of a polyethoxylated tridecanol surfactant. Bright red prints were obtained in each case.

## EXAMPLE 80

This example illustrates the preparation of a ferromagnetic dye toner containing a red disperse dye, a soft ferromagnetic component and an aqueous alkali-soluble resin, and the application thereof to paper.

A ferromagnetic toner was prepared by spray-drying a mixture containing 10% of polyvinyl acetate copolymer resin ("Gelva" C5-VIOM), 1% of C.I. Disperse Red 60, 3.2% of lignin sulfonate dispersant and 85.8% of Carbonyl Iron GS-6. The spray-dried toner was fluidized with 1% of Quso WR-82. The toner was used to develop the latent magnetic image on the surface of a continuously  $CrO_2$ -coated (220 microinches) (5.59  $\times 10^{-4}$  cm) aluminized "Mylar" polyester film as described in Example 1. The surface of the  $CrO_2$  film was magnetically structured into a 500 lines per inch (197 lines per cm) magnetic pattern using a magnetic write head and then imagewise demagnetized by exposure to a short burst from a Xenon lamp flashed through an image-bearing photographic transparency. The resultant latent magnetic image was manually decorated with toner particles and the toner decorated image was electrostatically transferred to paper and fused thereon as described in Example 1. A well-defined, background-free red print was obtained.

## EXAMPLE 81

A ferromagnetic toner containing 36% of polyvinyl acetate copolymer resin ("Gelva" C5-VIOM), 1% of C.I. Disperse Red 60, 3.2% of lignin sulfonate dispersant and 59.8% of Carbonyl Iron GS-6 was similarly prepared and applied to paper as described in Example 80. The results obtained were comparable.

TABLE I

| Ex. No. | Resin <sup>a</sup> | Toner Composition (Wt. %)    |                              | Dye                          | Other <sup>d</sup> | Resin      |                                                                         | Remarks <sup>e</sup> |
|---------|--------------------|------------------------------|------------------------------|------------------------------|--------------------|------------|-------------------------------------------------------------------------|----------------------|
|         |                    | Soft Mag. Comp. <sup>b</sup> | Hard Mag. Comp. <sup>c</sup> |                              |                    | Mag. Comp. | Resin                                                                   |                      |
| 4       | PVAC (28)          | Fe (34)                      | $Fe_3O_4$ (34)               | C.I. Disperse Yellow 54 (2)  | 2                  | 0.41       | HTP(PE) <sup>f,g</sup><br>DP(PE) <sup>f,g</sup><br>DP(Pap) <sup>f</sup> |                      |
| 5       | PVAC (29.1)        | Fe (34)                      | $Fe_3O_4$ (33)               | C.I. Disperse Blue 56 (1)    | 2.9                | 0.43       | DP(PE) <sup>h,f,i</sup>                                                 |                      |
| 6       | PVAC (26)          | Fe (28.7)                    | $Fe_3O_4$ (28.7)             | C.I. Disperse Blue 56 (4.3)  | 12.3               | 0.45       | DP(PE) <sup>h,f,i</sup>                                                 |                      |
| 7       | PVAC (23)          | Fe (23.1)                    | $Fe_3O_4$ (23.1)             | C.I. Disperse Blue 56 (7.6)  | 23.2               | 0.50       | DP(PE) <sup>h,f,i</sup>                                                 |                      |
| 8       | PVAC (20.5)        | Fe (19.2)                    | $Fe_3O_4$ (18.5)             | C.I. Disperse Blue 56 (10.3) | 31.5               | 0.54       | DP(PE) <sup>h,f,i</sup>                                                 |                      |
| 9       | PVAC (18.6)        | Fe (15.5)                    | $Fe_3O_4$ (15.5)             | C.I. Disperse Blue 56 (12.4) | 38                 | 0.60       | DP(PE) <sup>h,f,i</sup>                                                 |                      |
| 10      | PVAC (15.7)        | Fe (10.4)                    | $Fe_3O_4$ (10.4)             | C.I. Disperse Blue 56 (15.7) | 47.8               | 0.75       | DP(PE) <sup>h,f,i</sup>                                                 |                      |
| 11      | PVAC (13.5)        | Fe (6.8)                     | $Fe_3O_4$ (6.8)              | C.I. Disperse Blue 56 (18.0) | 54.9               | 1.0        | DP(PE) <sup>h,f,i</sup>                                                 |                      |
| 12      | PVAC (9.4)         | Fe (41.5)                    | $Fe_3O_4$ (41.5)             | C.I. Disperse Blue 56 (1.9)  | 5.7                | 0.11       | DP(PE) <sup>h,f,i</sup>                                                 |                      |
| 13      | PVAC (60)          | Fe (19)                      | $Fe_3O_4$ (20)               | C.I. Disperse Blue 56 (1)    | —                  | 1.54       | DP(PE) <sup>h,f,i</sup>                                                 |                      |
| 14      | PVAC (30)          | Fe (28)                      | $Fe_3O_4$ (27)               | C.I. Disperse Blue 56 (15)   | —                  | 0.55       | DP(PE) <sup>h,f,i</sup>                                                 |                      |
| 15      | PVAC (28.2)        | Fe (32)                      | $Fe_3O_4$ (32)               | C.I. Disperse Red 60 (1.9)   | 5.9                | 0.44       | DP(PE) <sup>h,f,i</sup>                                                 |                      |
| 16      | PAM (28.2)         | Fe (32)                      | $Fe_3O_4$ (32)               | C.I. Disperse Red 60 (1.9)   | 5.9                | 0.44       | DP(PE) <sup>h,f,i</sup>                                                 |                      |
| 17      | HPC (28.2)         | Fe (32)                      | $Fe_3O_4$ (32)               | C.I. Disperse Red 60 (1.9)   | 5.9                | 0.44       | DP(PE) <sup>h,f,i</sup>                                                 |                      |
| 18      | PVAC (45)          | None                         | $Fe_3O_4$ (46.9)             | C.I. Disperse Red 60 (1.9)   | 6.2                | 0.96       | DP(Ny) <sup>h,f,g</sup>                                                 |                      |
| 19      | PVAC (45)          | None                         | $Fe_3O_4$ (46.9)             | C.I. Disperse Red 60 (1.9)   | 6.2                | 0.96       | DP(Ny) <sup>h,f,g</sup>                                                 |                      |
| 20      | PVAC (60)          | None                         | $Fe_3O_4$ (35.8)             | C.I. Disperse Red 60 (1)     | 3.2                | 1.7        | DP(PE) <sup>h,f,i</sup>                                                 |                      |
| 21      | PVAC (30)          | None                         | $CrO_2$ (65.8)               | C.I. Disperse Red (1)        | 3.2                | 0.45       | DP(PE) <sup>h,f,i</sup>                                                 |                      |
| 22      | PVAC (30)          | Fe (32.8)                    | $CrO_2$ (33)                 | C.I. Disperse Red 60 (1)     | 3.2                | 0.45       | DP(PE) <sup>h,f,i</sup>                                                 |                      |
| 23      | PVAC (51.8)        | Fe (22)                      | $CrO_2$ (22)                 | C.I. Disperse Red 60 (1)     | 3.2                | 1.2        | DP(PE) <sup>h,f,i</sup>                                                 |                      |
| 24      | PVAC (61.8)        | Fe (17)                      | $CrO_2$ (17)                 | C.I. Disperse Red 60 (1)     | 3.2                | 1.8        | DP(PE) <sup>h,f,i</sup>                                                 |                      |
| 25      | PVAC (73.8)        | Fe (11)                      | $CrO_2$ (11)                 | C.I. Disperse Red 60 (1)     | 3.2                | 3.3        | DP(PE) <sup>h,f,i</sup>                                                 |                      |
| 26      | PVAC (29.4)        | Fe (33.3)                    | $Fe_3O_4$ (33.3)             | — (1.96)                     | 1.84               | 0.44       | DP(PE) <sup>h,f,g</sup><br>DP(PE) <sup>h,k,g</sup>                      |                      |
| 27      | PVAC (30)          | Fe (32)                      | $Fe_3O_4$ (32)               | — (2)                        | 4 <sup>l</sup>     | 0.47       | DP(PE) <sup>h,k,g</sup>                                                 |                      |

TABLE I-continued

| FERROMAGNETIC DISPERSE DYE TONERS CONTAINING WATER-SOLUBLE RESINS |                    |                              |                                     |                              |                    |            |                                                                                                                                                                                                                      |
|-------------------------------------------------------------------|--------------------|------------------------------|-------------------------------------|------------------------------|--------------------|------------|----------------------------------------------------------------------------------------------------------------------------------------------------------------------------------------------------------------------|
| Ex. No.                                                           | Resin <sup>a</sup> | Toner Composition (Wt. %)    |                                     |                              | Other <sup>d</sup> | Resin      | Remarks <sup>e</sup>                                                                                                                                                                                                 |
|                                                                   |                    | Soft Mag. Comp. <sup>b</sup> | Hard Mag. Comp. <sup>c</sup>        | Dye                          |                    | Mag. Comp. |                                                                                                                                                                                                                      |
| 28                                                                | PVAC (30)          | Fe (33)                      | Fe <sub>3</sub> O <sub>4</sub> (33) | <sup>s</sup> (2)             | 2                  | 0.45       | DP(PE) <sup>h,k,g</sup><br>DP(PE) <sup>h,p,g</sup><br>DP(PE) <sup>h,q,g</sup><br>DP(PE) <sup>h,j,g</sup><br>DP(PE) <sup>h,k,g</sup><br>DP(PE) <sup>h,p,g</sup><br>DP(PE) <sup>h,q,g</sup><br>DP(PE) <sup>h,j,g</sup> |
| 29                                                                | PVAC (30)          | Fe (31)                      | Fe <sub>3</sub> O <sub>4</sub> (31) | <sup>s</sup> (2)             | 6 <sup>m</sup>     | 0.48       | DP(PE) <sup>h,k,g</sup><br>DP(PE) <sup>h,j,g</sup><br>DP(PE) <sup>h,k,g</sup><br>DP(PE) <sup>h,j,g</sup><br>DP(PE) <sup>h,k,g</sup><br>DP(PE) <sup>h,j,g</sup><br>DP(PE) <sup>h,k,g</sup><br>DP(PE) <sup>h,j,g</sup> |
| 30                                                                | PVAC (30)          | Fe (30)                      | Fe <sub>3</sub> O <sub>4</sub> (30) | <sup>s</sup> (2)             | 8 <sup>n</sup>     | 0.50       | DP(PE) <sup>h,k,g</sup><br>DP(PE) <sup>h,j,g</sup><br>DP(PE) <sup>h,k,g</sup><br>DP(PE) <sup>h,j,g</sup><br>DP(PE) <sup>h,k,g</sup><br>DP(PE) <sup>h,j,g</sup><br>DP(PE) <sup>h,k,g</sup><br>DP(PE) <sup>h,j,g</sup> |
| 31                                                                | PVAC (30)          | Fe (29)                      | Fe <sub>3</sub> O <sub>4</sub> (29) | <sup>s</sup> (2)             | 10 <sup>o</sup>    | 0.52       | DP(PE) <sup>h,k,g</sup><br>DP(PE) <sup>h,j,g</sup><br>DP(PE) <sup>h,k,g</sup><br>DP(PE) <sup>h,j,g</sup><br>DP(PE) <sup>h,k,g</sup><br>DP(PE) <sup>h,j,g</sup><br>DP(PE) <sup>h,k,g</sup><br>DP(PE) <sup>h,j,g</sup> |
| 32                                                                | PVAC (30)          | Fe (23)                      | Fe <sub>3</sub> O <sub>4</sub> (22) | C.I. Disperse Blue 56 (25).  | —                  | 0.67       | DP(PE) <sup>h,f,i</sup>                                                                                                                                                                                              |
| 33                                                                | PVAC (30)          | Fe (34.6)                    | Fe <sub>3</sub> O <sub>4</sub> (35) | C.I. Disperse Blue 56 (0.10) | 0.3                | 0.48       | DP(PE) <sup>h,f,i</sup><br>DP(PE) <sup>h,f,i</sup>                                                                                                                                                                   |

TABLE II

| FERROMAGNETIC CATIONIC DYE TONERS CONTAINING WATER-SOLUBLE RESINS |                    |                              |                                       |                                          |                    |            |                                                           |
|-------------------------------------------------------------------|--------------------|------------------------------|---------------------------------------|------------------------------------------|--------------------|------------|-----------------------------------------------------------|
| Ex. No.                                                           | Resin <sup>a</sup> | Toner Composition (Wt. %)    |                                       |                                          | Other <sup>d</sup> | Resin      | Remarks <sup>e</sup>                                      |
|                                                                   |                    | Soft Mag. Comp. <sup>b</sup> | Hard Mag. Comp. <sup>c</sup>          | Dye                                      |                    | Mag. Comp. |                                                           |
| 38                                                                | PVAC (30)          | Fe (30)                      | Fe <sub>3</sub> O <sub>4</sub> (31)   | C.I. Basic Yellow 11 (2)<br>(C.I. 48055) | 7                  | 0.44       | DP(AMPE) <sup>h,u,q,f</sup><br>DP(PAN) <sup>h,u,v,i</sup> |
| 39                                                                | PVAC (30)          | Fe (29.6)                    | Fe <sub>3</sub> O <sub>4</sub> (30)   | C.I. Basic Red 14 (2)                    | 8.4                | 0.55       | DP(AMPE) <sup>h,u,q,f</sup><br>DP(PAN) <sup>h,u,v,i</sup> |
| 40                                                                | PVAC (30)          | Fe (31.4)                    | Fe <sub>3</sub> O <sub>4</sub> (31.5) | C.I. Basic Red 19 (2)                    | 5.1                | 0.48       | DP(AMPE) <sup>h,u,q,f</sup><br>DP(PAN) <sup>h,u,v,i</sup> |
| 41                                                                | HPC (30)           | Fe (29.6)                    | Fe <sub>3</sub> O <sub>4</sub> (30)   | C.I. Basic Red 14 (2)                    | 8.4                | 0.50       | DP(AMPE) <sup>h,q,f</sup><br>DP(AMPE) <sup>h,u,q,f</sup>  |
| 42                                                                | HPC (30)           | Fe (29.3)                    | Fe <sub>3</sub> O <sub>4</sub> (29.3) | C.I. Basic Red 14 (2)                    | 9.4 <sup>w</sup>   | 0.51       | DP(AMPE) <sup>h,q,f</sup><br>DP(PAN) <sup>h,v,i</sup>     |
| 43                                                                | PVAC (30)          | Fe (28.6)                    | Fe <sub>3</sub> O <sub>4</sub> (29)   | C.I. Basic Red 14 (2)                    | 10.4 <sup>x</sup>  | 0.52       | DP(AMPE) <sup>h,g,f</sup><br>DP(PAN) <sup>h,v,y</sup>     |

TABLE III

| FERROMAGNETIC ACID DYE TONERS CONTAINING WATER-SOLUBLE RESINS |                    |                              |                                       |                                        |                    |            |                                                      |
|---------------------------------------------------------------|--------------------|------------------------------|---------------------------------------|----------------------------------------|--------------------|------------|------------------------------------------------------|
| Ex. No.                                                       | Resin <sup>a</sup> | Toner Composition (Wt. %)    |                                       |                                        | Other <sup>d</sup> | Resin      | Remarks <sup>e</sup>                                 |
|                                                               |                    | Soft Mag. Comp. <sup>b</sup> | Hard Mag. Comp. <sup>c</sup>          | Dye                                    |                    | Mag. Comp. |                                                      |
| 45                                                            | PVAC (30)          | Fe (33)                      | Fe <sub>3</sub> O <sub>4</sub> (33.4) | C.I. Acid Yellow 174 (2)               | 1.6                | 0.45       | DP(Ny) <sup>h,u,v,h</sup><br>DP(Ny) <sup>h,v,y</sup> |
| 46                                                            | PAM (30)           | Fe (32.7)                    | Fe <sub>3</sub> O <sub>4</sub> (32.7) | C.I. Acid Red 151 (2)<br>(C.I. 26,900) | 2.6 <sup>z</sup>   | 0.46       | DP(Ny) <sup>h,v,i</sup>                              |
| 47                                                            | PAM (30)           | Fe (31.4)                    | Fe <sub>3</sub> O <sub>4</sub> (31.4) | C.I. Acid Blue 40 (2)                  | 5.2 <sup>z</sup>   | 0.48       | DP(Ny) <sup>h,v,y</sup>                              |
| 48                                                            | PVAC (28.3)        | Fe (32.2)                    | Fe <sub>3</sub> O <sub>4</sub> (32.2) | C.I. Acid Blue 40 (2.3)                | 5.0                | 0.44       | DP(Ny) <sup>h,u,v,i</sup><br>DP(Ny) <sup>h,v,y</sup> |
| 49                                                            | HPC (28.8)         | Fe (32.6)                    | Fe <sub>3</sub> O <sub>4</sub> (30.7) | C.I. Acid Blue 40 (1.9)                | 6.0 <sup>x</sup>   | 0.45       | DP(Ny) <sup>h,v,i</sup>                              |
| 50                                                            | PVAC (30)          | Fe (33)                      | Fe <sub>3</sub> O <sub>4</sub> (34)   | C.I. Acid Blue 40 (2)                  | 1 <sup>z</sup>     | 0.45       | DP(Ny) <sup>h,v,y</sup>                              |
| 51                                                            | PAM (30)           | Fe (33)                      | Fe <sub>3</sub> O <sub>4</sub> (33.4) | C.I. Acid Yellow 174 (2)               | 1.6 <sup>z</sup>   | 0.45       | DP(Ny) <sup>h,v,y</sup>                              |
| 52                                                            | PVAC (30)          | Fe (33)                      | Fe <sub>3</sub> O <sub>4</sub> (33)   | C.I. Acid Blue 127 (2)<br>(C.I. 61135) | 2                  | 0.45       | DP(Ny) <sup>h,v,y</sup>                              |
| 53                                                            | PAM (30)           | Fe (32)                      | Fe <sub>3</sub> O <sub>4</sub> (33)   | C.I. Acid Blue 127 (2)                 | 3 <sup>z</sup>     | 0.46       | DP(Ny) <sup>h,v,y</sup>                              |

TABLE IV

| FERROMAGNETIC CATIONIC-DISPERSE DYE TONERS CONTAINING WATER-SOLUBLE RESINS |                    |                              |                                     |                                                       |                    |            |                                                                                          |
|----------------------------------------------------------------------------|--------------------|------------------------------|-------------------------------------|-------------------------------------------------------|--------------------|------------|------------------------------------------------------------------------------------------|
| Ex. No.                                                                    | Resin <sup>a</sup> | Toner Composition (Wt. %)    |                                     |                                                       | Other <sup>d</sup> | Resin      | Remarks <sup>e</sup>                                                                     |
|                                                                            |                    | Soft Mag. Comp. <sup>b</sup> | Hard Mag. Comp. <sup>c</sup>        | Dye                                                   |                    | Mag. Comp. |                                                                                          |
| 65                                                                         | PVAC (30)          | Fe (33)                      | Fe <sub>3</sub> O <sub>4</sub> (33) | C.I. Basic Yellow 21<br>and 1,5 NDS (2) <sup>aa</sup> | 2                  | 0.45       | DP(AMPE) <sup>h,u,g,f</sup><br>DP(PAN) <sup>h,u,v,i</sup>                                |
| 66                                                                         | PVAC (30)          | Fe (33)                      | Fe <sub>3</sub> O <sub>4</sub> (33) | C.I. Basic Red 14<br>and 1,5 NDS (2) <sup>aa</sup>    | 2                  | 0.45       | DP(AMPE) <sup>h,u,g,f</sup><br>DP(PAN) <sup>h,u,v,i</sup><br>DP(Acet) <sup>h,u,v,i</sup> |
| 67                                                                         | PVAC (30)          | Fe (33)                      | Fe <sub>3</sub> O <sub>4</sub> (33) | C.I. Basic Blue 69<br>and 1,5 NDS (2) <sup>aa</sup>   | 2                  | 0.45       | DP(AMPE) <sup>h,u,g,f</sup><br>DP(PAN) <sup>h,u,v,i</sup>                                |
| 68                                                                         | PVAC (30)          | Fe (33)                      | Fe <sub>3</sub> O <sub>4</sub> (33) | C.I. Basic Blue 77<br>and 2,4-DNBS (2) <sup>bb</sup>  | 2                  | 0.45       | DP(AMPE) <sup>h,u,g,f</sup><br>DP(PAN) <sup>h,u,v,i</sup>                                |

TABLE V

| Example No. | Resin <sup>a</sup> | Toner Composition (Wt. %)    |                                     | Chemical Resist Agent | Resin Mag. Comp. | Remarks <sup>c</sup>                                                                |
|-------------|--------------------|------------------------------|-------------------------------------|-----------------------|------------------|-------------------------------------------------------------------------------------|
|             |                    | Soft Mag. Comp. <sup>b</sup> | Hard Mag. Comp. <sup>c</sup>        |                       |                  |                                                                                     |
| 70          | PVAC (30)          | Fe (34)                      | Fe <sub>3</sub> O <sub>4</sub> (34) | (2) <sup>cc</sup>     | 0.44             | DP(Ny) <sup>h,dd,ee</sup><br>DP(Ny) <sup>h,dd,ff</sup><br>DP(Ny) <sup>h,dd,gg</sup> |
| 71          | PVAC (30)          | Fe (33)                      | Fe <sub>3</sub> O <sub>4</sub> (33) | (4) <sup>cc</sup>     | 0.45             | DP(Ny) <sup>h,dd,ee</sup><br>DP(Ny) <sup>h,dd,ff</sup><br>DP(Ny) <sup>h,dd,gg</sup> |
| 72          | PVAC (30)          | Fe (32)                      | Fe <sub>3</sub> O <sub>4</sub> (32) | (6) <sup>cc</sup>     | 0.47             | DP(Ny) <sup>h,dd,ee</sup><br>DP(Ny) <sup>h,dd,ff</sup><br>DP(Ny) <sup>h,dd,gg</sup> |
| 73          | PVAC (30)          | Fe (31)                      | Fe <sub>3</sub> O <sub>4</sub> (31) | (8) <sup>cc</sup>     | 0.48             | DP(Ny) <sup>h,dd,ee</sup><br>DP(Ny) <sup>h,dd,ff</sup><br>DP(Ny) <sup>h,dd,gg</sup> |
| 74          | PVAC (30)          | None                         | CrO <sub>2</sub> (69)               | (1) <sup>cc</sup>     | 0.43             | DP(Ny) <sup>h,dd,ff</sup><br>DP(Ny) <sup>h,dd,gg</sup>                              |

TABLE VI

## DEFINITIONS OF SYMBOLS USED IN TABLES I-V

<sup>a</sup>PVAC = polyvinyl acetate copolymer ("Gelva" CS-VIOM); PAM = polyamide polymer (TPX-1002); HPC = hydroxypropylcellulose polymer (Klucel LF)

<sup>b</sup>All iron is Carbonyl Iron GS-6

<sup>c</sup>All Fe<sub>3</sub>O<sub>4</sub> is "Mapico" Black Iron Oxide

<sup>d</sup>Dispersants and/or inorganic diluents

<sup>e</sup>HTP = heat transfer printed; DP = directly printed; PE = polyester; Ny = nylon;

Pap = paper; AMPE - acid-modified polyester; PAN - polyacrylonitrile; Acet - cellulose acetate

<sup>f</sup>Heat fixed at 205° C for 40 seconds and 1.5 psig (0.11 kg per sq cm gauge)

<sup>g</sup>Scoured in hot water (65° C) containing "Lakeseal" detergent

<sup>h</sup>Steam fused at 100° C and 1 atm for 10 to 15 seconds

<sup>i</sup>Scoured in 2 parts/liter sodium hydroxide, 2 parts/liter soda caustic and 2 parts/liter polyethoxylated tridecanol surfactant at 65° C

<sup>j</sup>Hot air fixation at 205° C for 100 seconds

<sup>k</sup>Heat fixation at 205° C for 100 seconds and 1.5 psig (0.11 kg per sq cm gauge)

<sup>l</sup>Includes 2% by weight of benzanilide carrier

<sup>m</sup>Includes 4% by weight of benzanilide carrier

<sup>n</sup>Includes 6% by weight of benzanilide carrier

<sup>o</sup>Includes 8% by weight of benzanilide carrier

<sup>p</sup>High temperature steam fixation at 182° C for 8 minutes

<sup>q</sup>High pressure steam fixation at 22 psig (1.55 kg per sq cm gauge) for 1 hour



<sup>aa</sup>Infrared fusion at 160-170° C

<sup>bb</sup>Fabric sprayed with 50% aqueous citric acid before fixation

<sup>cc</sup>Cottage-steamed at 7 psig (0.49 kg per sq cm gauge) for 1 hour

<sup>dd</sup>Includes 1% by weight of citric acid

<sup>ee</sup>Includes 2% by weight of citric acid

<sup>ff</sup>Scoured at 60° C with 2 parts/liter of polyethoxylated oleyl alcohol and 2 parts/liter of alkyltrimethylammonium bromide surfactants

<sup>gg</sup>Includes 1% by weight of ammonium oxalate

<sup>hh</sup>1,5 NDS = 1,5-naphthalenedisulfonate

<sup>ii</sup>2,4 DNBS = 2,4-dinitrobenzenesulfonate

<sup>cc</sup>



<sup>dd</sup>High temperature steam fixation at 182° C for 20 minutes

<sup>ee</sup>Overdyed with 0.5% owf of dye (D) of Table VII

<sup>ff</sup>Overdyed with 0.5% owf of dye (E) of Table VII

<sup>gg</sup>Overdyed with 0.5% each of dye (D) and dye (E) of Table VII

TABLE VII



I claim:

1. Ferromagnetic toner for magnetically printing a substrate, said toner comprising:
  - (a) at least one ferromagnetic component;
  - (b) at least one member of the group consisting of dye and chemical treating agent, said agent being selected from the group consisting of flame-retarding agent, biocide, ultraviolet light absorber, fluorescent brightener, dyeability modifier, soil-release agent and water-proofing agent; and
  - (c) a readily fusible, aqueous scour-removable water-soluble or water-solubilizable resin which substantially encapsulates (a) and (b).
2. Ferromagnetic toner of claim 1 comprising, based on the total weight of (a), (b) and (c), 14 to 83% of (a), 0.10 to 25% of (b) and 9 to 74% of (c) and having a resin to ferromagnetic component ratio of 0.11 to 3.3.
3. Ferromagnetic toner of claim 2 comprising 55 to 70% of (a), 0.10 to 15% of (b) and 30 to 40% of (c) and having a resin to ferromagnetic component ratio of 0.40 to 1.0.
4. Ferromagnetic toner of claim 1 wherein the ferromagnetic component consists of hard magnetic particles.

5. Ferromagnetic toner of claim 4 wherein the hard magnetic particles are  $Fe_3O_4$  particles.
6. Ferromagnetic toner of claim 4 wherein the hard magnetic particles are chromium dioxide particles.
7. Ferromagnetic toner of claim 4 wherein the hard magnetic particles consist of an alloy of  $Fe_3O_4$  and cobalt.
8. Ferromagnetic toner of claim 4 wherein the hard magnetic particles consist of an alloy of  $Fe_3O_4$  and nickel.
9. Ferromagnetic toner of claim 1 wherein the ferromagnetic component consists of a binary mixture of hard and soft magnetic particles.
10. Ferromagnetic toner of claim 9 wherein the hard and soft magnetic particles are  $Fe_3O_4$  particles and iron particles, respectively.
11. Ferromagnetic toner of claim 9 wherein the hard and soft magnetic particles are chromium dioxide particles and iron particles, respectively.
12. Ferromagnetic toner of claim 1 wherein the dye is a disperse dye.
13. Ferromagnetic toner of claim 1 wherein the dye is a cationic dye.
14. Ferromagnetic toner of claim 1 wherein the dye is an acid dye.
15. Ferromagnetic toner of claim 1 wherein the dye is a premetalized acid dye.
16. Ferromagnetic toner of claim 1 wherein the dye is a vat dye.
17. Ferromagnetic toner of claim 1 wherein the dye is a sulfur dye.
18. Ferromagnetic toner of claim 1 wherein the dye is a fiber-reactive dye.
19. Ferromagnetic toner of claim 1 wherein the dye is a mixture of a disperse dye and a fiber-reactive dye.
20. Ferromagnetic toner of claim 1 wherein the dye is a salt of a dye cation and an arylsulfonate anion.
21. Ferromagnetic toner of claim 1 wherein the chemical treating agent is a fluorescent brightening agent.
22. Ferromagnetic toner of claim 1 wherein the chemical treating agent is a dyeability modifier.
23. Ferromagnetic toner of claim 1 wherein the chemical treating agent is a flame retarding agent.
24. Ferromagnetic toner of claim 1 wherein the chemical treating agent is a biocidal agent.
25. Ferromagnetic toner of claim 1 wherein the chemical treating agent is an ultraviolet light absorbing agent.
26. Ferromagnetic toner of claim 1 wherein the chemical treating agent is a soil-release agent.
27. Ferromagnetic toner of claim 1 wherein the chemical treating agent is a water-proofing agent.
28. Ferromagnetic toner of claim 1 wherein the resin is a natural, modified natural or synthetic resin.
29. Ferromagnetic toner of claim 1 wherein the resin is a thermoplastic resin.
30. Ferromagnetic toner of claim 1 wherein the resin can be removed by an aqueous alkaline scour in less than five minutes at less than 90° C.
31. Ferromagnetic toner of claim 1 wherein the resin is an adduct of rosin, a dicarboxylic acid or anhydride, a polymeric fatty acid and an alkylene polyamide.
32. Ferromagnetic toner of claim 1 wherein the resin is a hydroxypropylcellulose prepared by reacting 3.5 to 4.2 moles of propylene oxide per D-glucopyranosyl unit of the cellulose.

33. Ferromagnetic toner of claim 1 wherein the resin is a polyvinyl acetate copolymer having a free carboxy group content equivalent to 0.002 to 0.01 equivalent of ammonium hydroxide per gram of copolymer.

34. Ferromagnetic toner of claim 1 containing from 0.01 to 5% by weight, based on total toner weight, of a free-flow agent.

35. Ferromagnetic toner of claim 34 containing from 0.01 to 0.4% of a free flow agent, which agent is an alumina or fumed silica.

36. Ferromagnetic toner of claim 12 wherein there is also present a benzanilide dye carrier.

37. Ferromagnetic toner of claim 12 wherein there is also present a butyl benzoate dye carrier.

38. Ferromagnetic toner of claim 12 wherein there is also present a  $\beta$ -naphthol dye carrier.

39. Ferromagnetic toner of claim 12 wherein there is also present an o-phenylphenol dye carrier.

40. Ferromagnetic toner of claim 12 wherein there is also present a lignin sulfonate dispersant.

41. Ferromagnetic toner of claim 12 wherein there is also present a dispersant which is a salt of a sulfonated naphthalene-formaldehyde condensate.

42. Ferromagnetic toner of claim 1 wherein there is also present a static-reducing cationic surfactant.

43. Ferromagnetic toner of claim 13 wherein there is also present citric acid.

44. Ferromagnetic toner of claim 14 wherein there is also present citric acid.

5 45. Ferromagnetic toner of claim 14 wherein there is also present ammonium oxalate.

46. Ferromagnetic toner of claim 12 wherein there is also present a sodium chlorate oxidizing agent.

10 47. Ferromagnetic toner of claim 1 having a particle size within the range of 2 to 100 microns.

48. Ferromagnetic toner of claim 47 wherein the particle size range is 10 to 25 microns.

49. Ferromagnetic toner of claim 1 having a particle size of less than 74 microns.

15 50. Ferromagnetic toner of claim 1 wherein the ferromagnetic component consists of soft magnetic particles.

51. Ferromagnetic toner of claim 50 wherein the soft magnetic particles are iron particles.

20 52. Ferromagnetic toner of claim 1 which is useful for magnetically printing a dyeable fabric substrate and which includes as a component thereof a dye.

53. Ferromagnetic toner of claim 52 wherein the dye is a disperse dye for dyeing a polyester fabric substrate.

25 54. Ferromagnetic toner of claim 53 wherein the resin is aqueous alkaline scour-removable from the polyester fabric substrate.

\* \* \* \* \*